



US012031400B2

(12) **United States Patent**  
**Doud et al.**

(10) **Patent No.:** **US 12,031,400 B2**  
(45) **Date of Patent:** **\*Jul. 9, 2024**

(54) **FLUID ACTIVATED DISINTEGRATING METAL SYSTEM**

(71) Applicant: **Terves, LLC**, Euclid, OH (US)

(72) Inventors: **Brian Doud**, Euclid, OH (US); **Andrew Sherman**, Euclid, OH (US); **Nicholas Farkas**, Euclid, OH (US); **Brian Werry**, Euclid, OH (US)

(73) Assignee: **Terves, LLC**, Euclid, OH (US)

(\*) Notice: Subject to any disclaimer, the term of this patent is extended or adjusted under 35 U.S.C. 154(b) by 0 days.

This patent is subject to a terminal disclaimer.

(21) Appl. No.: **18/110,183**

(22) Filed: **Feb. 15, 2023**

(65) **Prior Publication Data**

US 2023/0193713 A1 Jun. 22, 2023

**Related U.S. Application Data**

(63) Continuation of application No. 17/124,723, filed on Dec. 17, 2020, now Pat. No. 11,613,952, which is a (Continued)

(51) **Int. Cl.**  
*E21B 29/02* (2006.01)  
*C06B 45/18* (2006.01)

(Continued)

(52) **U.S. Cl.**  
CPC ..... *E21B 29/02* (2013.01); *C06B 45/18* (2013.01); *C06B 45/32* (2013.01); *E21B 31/002* (2013.01); (Continued)

(58) **Field of Classification Search**  
CPC ..... E21B 29/00; E21B 29/02; E21B 31/002; C06B 45/18; C06B 45/32

See application file for complete search history.

(56) **References Cited**

**U.S. PATENT DOCUMENTS**

1,468,905 A 7/1923 Herman  
1,558,066 A 10/1925 Veazey et al.

(Continued)

**FOREIGN PATENT DOCUMENTS**

CA 2783241 6/2011  
CA 2783346 6/2011

(Continued)

**OTHER PUBLICATIONS**

Hemanth, "Fracture Behavior of Cryogenically solidified aluminum-alloy reinforced with Nano-ZrO<sub>2</sub> Metal Matrix Composites (CNMMCs)", Journal of Chemical Engineering and Materials Science, vol. 2(8), pp. 110-121 (Aug. 2011).

(Continued)

*Primary Examiner* — Kristyn A Hall

(74) *Attorney, Agent, or Firm* — UB Greensfelder LLP;  
Brian E. Turung

(57) **ABSTRACT**

An engineered composite system designed to be passive or inert under one set of conditions, but becomes active when exposed to a second set of conditions. This system can include a dissolving or disintegrating core, and a surface coating that has higher strength or which only dissolves under certain temperature and pH conditions, or in selected fluids. These reactive materials are useful for oil and gas completions and well stimulation processes, enhanced oil and gas recovery operations, as well as in defensive and mining applications requiring high energy density and good mechanical properties, but which can be stored and used for long periods of time without degradation.

**9 Claims, 2 Drawing Sheets**



**Related U.S. Application Data**

continuation of application No. 16/110,550, filed on Aug. 23, 2018, now Pat. No. 11,365,164, which is a continuation of application No. 14/627,189, filed on Feb. 20, 2015, now Pat. No. 10,150,713.

(60) Provisional application No. 62/054,597, filed on Sep. 24, 2014, provisional application No. 61/942,870, filed on Feb. 21, 2014.

**(51) Int. Cl.**

**C06B 45/32** (2006.01)  
**E21B 31/00** (2006.01)  
**E21B 33/12** (2006.01)

**(52) U.S. Cl.**

CPC ..... **E21B 33/12** (2013.01); **Y10T 428/12729** (2015.01); **Y10T 428/31605** (2015.04); **Y10T 428/31692** (2015.04)

**(56) References Cited****U.S. PATENT DOCUMENTS**

|             |         |                      |             |         |                       |
|-------------|---------|----------------------|-------------|---------|-----------------------|
| 1,880,614 A | 10/1932 | Wetherill et al.     | 3,823,045 A | 7/1974  | Hielema               |
| 2,352,993 A | 7/1933  | Albertson            | 3,878,889 A | 4/1975  | Seabourn              |
| 2,011,613 A | 8/1935  | Brown et al.         | 3,894,850 A | 7/1975  | Kovalchuk et al.      |
| 2,094,578 A | 10/1937 | Blumenthal et al.    | 3,924,677 A | 12/1975 | Prenner et al.        |
| 2,189,697 A | 2/1940  | Baker                | 3,957,483 A | 5/1976  | Suzuki                |
| 2,222,233 A | 11/1940 | Mize                 | 4,010,583 A | 3/1977  | Highberg              |
| 2,225,143 A | 12/1940 | Baker et al.         | 4,039,717 A | 8/1977  | Titus                 |
| 2,238,895 A | 4/1941  | Gage                 | 4,050,529 A | 9/1977  | Tagirov et al.        |
| 2,261,292 A | 11/1941 | Salnikov             | 4,157,732 A | 6/1979  | Fonner                |
| 2,294,648 A | 9/1942  | Ansel et al.         | 4,248,307 A | 2/1981  | Silberman et al.      |
| 2,301,624 A | 11/1942 | Holt                 | 4,264,362 A | 4/1981  | Serveg et al.         |
| 2,394,843 A | 2/1946  | Cook et al.          | 4,284,137 A | 8/1981  | Taylor                |
| 2,672,199 A | 3/1954  | McKenna              | 4,292,377 A | 9/1981  | Petersen et al.       |
| 2,753,941 A | 7/1956  | Hebard et al.        | 4,368,788 A | 1/1983  | Drake                 |
| 2,754,910 A | 7/1956  | Derrick et al.       | 4,372,384 A | 2/1983  | Kinney                |
| 2,933,136 A | 4/1960  | Ayers et al.         | 4,373,584 A | 2/1983  | Silberman et al.      |
| 2,983,634 A | 5/1961  | Budininkas et al.    | 4,373,952 A | 2/1983  | Parent                |
| 3,057,405 A | 10/1962 | Mallinger            | 4,374,543 A | 2/1983  | Richardson            |
| 3,066,391 A | 12/1962 | Vordahl et al.       | 4,384,616 A | 5/1983  | Dellinger             |
| 3,106,959 A | 10/1963 | Huitt et al.         | 4,395,440 A | 7/1983  | Abe et al.            |
| 3,142,338 A | 7/1964  | Brown                | 4,399,871 A | 8/1983  | Adkins et al.         |
| 3,152,009 A | 10/1964 | DeLong               | 4,407,368 A | 10/1983 | Erbstoesser           |
| 3,180,728 A | 4/1965  | Pryor et al.         | 4,422,508 A | 12/1983 | Rutledge, Jr. et al.  |
| 3,180,778 A | 4/1965  | Rinderspacher et al. | 4,450,136 A | 5/1984  | Dudek et al.          |
| 3,196,949 A | 7/1965  | Thomas               | 4,452,311 A | 6/1984  | Speegle et al.        |
| 3,226,314 A | 12/1965 | Wellington et al.    | 4,475,729 A | 10/1984 | Costigan              |
| 3,242,988 A | 3/1966  | McGuire, Jr. et al.  | 4,498,543 A | 2/1985  | Pye et al.            |
| 3,295,935 A | 1/1967  | Pflumm et al.        | 4,499,048 A | 2/1985  | Hanejko               |
| 3,298,440 A | 1/1967  | Current              | 4,499,049 A | 2/1985  | Hanejko               |
| 3,316,748 A | 5/1967  | Lang et al.          | 4,524,825 A | 6/1985  | Fore                  |
| 3,326,291 A | 6/1967  | Zandemer             | 4,526,840 A | 7/1985  | Jerabek               |
| 3,347,714 A | 10/1967 | Broverman et al.     | 4,534,414 A | 8/1985  | Pringle               |
| 3,385,696 A | 5/1968  | Hitchcock et al.     | 4,539,175 A | 9/1985  | Lichti et al.         |
| 3,390,724 A | 7/1968  | Caldwell             | 4,554,986 A | 11/1985 | Jones                 |
| 3,395,758 A | 8/1968  | Kelly et al.         | 4,619,699 A | 10/1986 | Petkovic-Luton et al. |
| 3,406,101 A | 10/1968 | Kilpatrick           | 4,640,354 A | 2/1987  | Boisson               |
| 3,416,918 A | 12/1968 | Roberts              | 4,648,901 A | 3/1987  | Murray et al.         |
| 3,434,539 A | 3/1969  | Merritt              | 4,655,852 A | 4/1987  | Rallis                |
| 3,445,148 A | 5/1969  | Harris et al.        | 4,664,962 A | 5/1987  | DesMarais, Jr.        |
| 3,445,731 A | 5/1969  | Saeki et al.         | 4,668,470 A | 5/1987  | Gilman et al.         |
| 3,465,181 A | 9/1969  | Colby et al.         | 4,673,549 A | 6/1987  | Ecer                  |
| 3,489,218 A | 1/1970  | Means                | 4,674,572 A | 6/1987  | Gallus                |
| 3,513,230 A | 5/1970  | Rhees et al.         | 4,678,037 A | 7/1987  | Smith                 |
| 3,600,163 A | 8/1971  | Badia et al.         | 4,706,753 A | 11/1987 | Weston                |
| 3,602,305 A | 8/1971  | Kisling              | 4,708,202 A | 11/1987 | Ohkochi et al.        |
| 3,637,446 A | 1/1972  | Elliott et al.       | 4,708,208 A | 11/1987 | Sukup et al.          |
| 3,645,331 A | 2/1972  | Maurer et al.        | 4,709,761 A | 12/1987 | Halbardier            |
| 3,660,049 A | 5/1972  | Benjamin             | 4,714,116 A | 12/1987 | Setterberg, Jr.       |
| 3,765,484 A | 10/1973 | Hamby, Jr. et al.    | 4,716,964 A | 1/1988  | Brunner               |
| 3,768,563 A | 10/1973 | Blount               | 4,719,971 A | 1/1988  | Erbstoesser et al.    |
| 3,775,823 A | 12/1973 | Adolph et al.        | 4,721,159 A | 1/1988  | Knieriemen            |
| 3,816,080 A | 6/1974  | Bomford et al.       | 4,738,599 A | 4/1988  | Paliwal               |
|             |         |                      | 4,741,973 A | 5/1988  | Del Corso et al.      |
|             |         |                      | 4,768,588 A | 5/1988  | Weston                |
|             |         |                      | 4,775,598 A | 10/1988 | Ohkochi et al.        |
|             |         |                      | 4,784,226 A | 11/1988 | Shilling              |
|             |         |                      | 4,805,699 A | 12/1988 | Condit et al.         |
|             |         |                      | 4,817,725 A | 12/1988 | Kupsa                 |
|             |         |                      | 4,834,184 A | 1/1989  | Jaeckel               |
|             |         |                      | 4,835,056 A | 1/1989  | Wyatt                 |
|             |         |                      | 4,869,324 A | 2/1989  | Halbardier            |
|             |         |                      | 4,869,325 A | 4/1989  | Jenkins               |
|             |         |                      | 4,875,948 A | 5/1989  | Streich et al.        |
|             |         |                      | 4,880,059 A | 11/1989 | Owens                 |
|             |         |                      | 4,889,187 A | 12/1989 | Johnson et al.        |
|             |         |                      | 4,890,675 A | 1/1990  | Hoffman               |
|             |         |                      | 4,901,794 A | 2/1990  | Holder                |
|             |         |                      | 4,909,320 A | 3/1990  | Hebert et al.         |
|             |         |                      | 4,916,029 A | 4/1990  | Nagle et al.          |
|             |         |                      | 4,917,966 A | 4/1990  | Wilde et al.          |
|             |         |                      | 4,921,664 A | 5/1990  | Couper                |
|             |         |                      | 4,929,415 A | 5/1990  | Okazaki               |
|             |         |                      | 4,932,474 A | 6/1990  | Schroeder, Jr. et al. |

(56)

## References Cited

## U.S. PATENT DOCUMENTS

|             |         |                    |             |         |                    |
|-------------|---------|--------------------|-------------|---------|--------------------|
| 4,934,459 A | 6/1990  | Baugh et al.       | 5,454,430 A | 10/1995 | Kennedy et al.     |
| 4,938,309 A | 7/1990  | Emdy               | 5,456,317 A | 10/1995 | Hood et al.        |
| 4,938,809 A | 7/1990  | Das et al.         | 5,456,327 A | 10/1995 | Denton et al.      |
| 4,944,351 A | 7/1990  | Eriksen et al.     | 5,464,062 A | 11/1995 | Blizzard, Jr.      |
| 4,949,788 A | 8/1990  | Szarka et al.      | 5,472,048 A | 12/1995 | Kennedy            |
| 4,952,902 A | 8/1990  | Kawaguchi et al.   | 5,474,131 A | 12/1995 | Jordan, Jr. et al. |
| 4,975,412 A | 12/1990 | Okazaki et al.     | 5,476,632 A | 12/1995 | Shivanath et al.   |
| 4,977,958 A | 12/1990 | Miller             | 5,477,923 A | 12/1995 | Jordan, Jr. et al. |
| 4,981,177 A | 1/1991  | Carmody et al.     | 5,479,986 A | 1/1996  | Gano et al.        |
| 4,986,361 A | 1/1991  | Mueller et al.     | 5,494,538 A | 2/1996  | Kirillov et al.    |
| 4,997,622 A | 3/1991  | Regazzoni et al.   | 5,506,055 A | 4/1996  | Dorfman et al.     |
| 5,006,044 A | 4/1991  | Walker, Sr. et al. | 5,507,439 A | 4/1996  | Story              |
| 5,010,955 A | 4/1991  | Springer           | 5,511,620 A | 4/1996  | Baugh et al.       |
| 5,036,921 A | 8/1991  | Pittard et al.     | 5,524,699 A | 6/1996  | Cook               |
| 5,048,611 A | 9/1991  | Cochran            | 5,526,880 A | 6/1996  | Jordan, Jr. et al. |
| 5,049,165 A | 9/1991  | Tselesin           | 5,526,881 A | 6/1996  | Martin et al.      |
| 5,061,323 A | 10/1991 | DeLucchia          | 5,529,746 A | 6/1996  | Knoss et al.       |
| 5,063,775 A | 11/1991 | Walker, Sr. et al. | 5,531,735 A | 7/1996  | Thompson           |
| 5,073,207 A | 12/1991 | Faure et al.       | 5,533,573 A | 7/1996  | Jordan, Jr. et al. |
| 5,074,361 A | 12/1991 | Brisco et al.      | 5,536,485 A | 7/1996  | Kume et al.        |
| 5,076,869 A | 12/1991 | Bourell et al.     | 5,552,110 A | 9/1996  | Iba                |
| 5,084,088 A | 1/1992  | Okazaki            | 5,558,153 A | 9/1996  | Holcombe et al.    |
| 5,087,304 A | 2/1992  | Chang et al.       | 5,601,924 A | 2/1997  | Beane et al.       |
| 5,090,480 A | 2/1992  | Pittard et al.     | 5,607,017 A | 3/1997  | Owens et al.       |
| 5,095,988 A | 3/1992  | Bode               | 5,623,993 A | 4/1997  | Van Buskirk et al. |
| 5,103,911 A | 4/1992  | Heijnen            | 5,623,994 A | 4/1997  | Robinson           |
| 5,106,702 A | 4/1992  | Walker et al.      | 5,641,023 A | 6/1997  | Ross et al.        |
| 5,117,915 A | 6/1992  | Mueller et al.     | 5,636,691 A | 7/1997  | Hendrickson et al. |
| 5,143,795 A | 9/1992  | Das et al.         | 5,647,444 A | 7/1997  | Williams           |
| 5,161,614 A | 11/1992 | Wu et al.          | 5,665,289 A | 9/1997  | Chung et al.       |
| 5,171,734 A | 12/1992 | Sanjurjo et al.    | 5,677,372 A | 10/1997 | Yamamoto et al.    |
| 5,178,216 A | 1/1993  | Giroux et al.      | 5,685,372 A | 11/1997 | Gano               |
| 5,181,571 A | 1/1993  | Mueller et al.     | 5,701,576 A | 12/1997 | Fujita et al.      |
| 5,183,631 A | 2/1993  | Kugimiya et al.    | 5,707,214 A | 1/1998  | Schmidt            |
| 5,188,182 A | 2/1993  | Echols, III et al. | 5,709,269 A | 1/1998  | Head               |
| 5,188,183 A | 2/1993  | Hopmann et al.     | 5,720,344 A | 2/1998  | Newman             |
| 5,204,055 A | 4/1993  | Sachs et al.       | 5,722,033 A | 2/1998  | Carden             |
| 5,222,867 A | 6/1993  | Walker, Sr. et al. | 5,728,195 A | 3/1998  | Eastman et al.     |
| 5,226,483 A | 7/1993  | Williamson, Jr.    | 5,765,639 A | 6/1998  | Muth               |
| 5,228,518 A | 7/1993  | Wilson et al.      | 5,767,562 A | 6/1998  | Yamashita          |
| 5,234,055 A | 8/1993  | Cornette           | 5,772,735 A | 6/1998  | Sehgal et al.      |
| 5,238,646 A | 8/1993  | Tarcy et al.       | 5,782,305 A | 7/1998  | Hicks              |
| 5,240,495 A | 8/1993  | Dieckmann et al.   | 5,797,454 A | 8/1998  | Hipp               |
| 5,240,742 A | 8/1993  | Johnson et al.     | 5,820,608 A | 10/1998 | Luzio et al.       |
| 5,252,365 A | 10/1993 | White              | 5,826,652 A | 10/1998 | Tapp               |
| 5,253,714 A | 10/1993 | Davis et al.       | 5,826,661 A | 10/1998 | Parker et al.      |
| 5,271,468 A | 12/1993 | Streich et al.     | 5,829,520 A | 11/1998 | Johnson            |
| 5,273,569 A | 12/1993 | Gilman et al.      | 5,836,396 A | 11/1998 | Norman             |
| 5,282,509 A | 2/1994  | Schurr, III        | 5,857,521 A | 1/1999  | Ross et al.        |
| 5,285,798 A | 2/1994  | Banerjee et al.    | 5,881,816 A | 3/1999  | Wright             |
| 5,292,478 A | 3/1994  | Scorey             | 5,896,819 A | 4/1999  | Turila et al.      |
| 5,293,940 A | 3/1994  | Hromas et al.      | 5,902,424 A | 5/1999  | Fujita et al.      |
| 5,304,260 A | 4/1994  | Aikawa et al.      | 5,934,372 A | 8/1999  | Muth               |
| 5,304,588 A | 4/1994  | Boysen et al.      | 5,941,309 A | 8/1999  | Appleton           |
| 5,309,874 A | 5/1994  | Willermet et al.   | 5,960,881 A | 10/1999 | Allamon et al.     |
| 5,310,000 A | 5/1994  | Arterbury et al.   | 5,964,965 A | 10/1999 | Schulz et al.      |
| 5,316,598 A | 5/1994  | Chang et al.       | 5,894,007 A | 11/1999 | Yuan et al.        |
| 5,318,746 A | 6/1994  | Lashmore et al.    | 5,980,602 A | 11/1999 | Carden             |
| 5,336,466 A | 8/1994  | Iba                | 5,985,466 A | 11/1999 | Atarashi et al.    |
| 5,342,576 A | 8/1994  | Whitehead          | 5,988,287 A | 11/1999 | Jordan, Jr. et al. |
| 5,352,522 A | 10/1994 | Kugimiya et al.    | 5,990,051 A | 11/1999 | Ischy et al.       |
| 5,380,473 A | 1/1995  | Bogue et al.       | 5,992,452 A | 11/1999 | Nelson, II         |
| 5,387,380 A | 2/1995  | Cima et al.        | 5,992,520 A | 11/1999 | Schultz et al.     |
| 5,392,860 A | 2/1995  | Ross               | 6,007,314 A | 12/1999 | Nelson, II         |
| 5,394,236 A | 2/1995  | Murnick            | 6,024,915 A | 2/2000  | Kume et al.        |
| 5,394,941 A | 3/1995  | Venditto et al.    | 6,030,637 A | 2/2000  | Whitehead          |
| 5,398,754 A | 3/1995  | Dinhoble           | 6,032,735 A | 3/2000  | Echols             |
| 5,407,011 A | 4/1995  | Layton             | 6,033,622 A | 3/2000  | Maruyama           |
| 5,409,555 A | 4/1995  | Fujita et al.      | 6,036,777 A | 3/2000  | Sachs              |
| 5,411,082 A | 5/1995  | Kennedy            | 6,036,792 A | 3/2000  | Chu et al.         |
| 5,417,285 A | 5/1995  | Van Buskirk et al. | 6,040,087 A | 3/2000  | Kawakami           |
| 5,425,424 A | 6/1995  | Reinhardt et al.   | 6,047,773 A | 4/2000  | Zeltmann et al.    |
| 5,427,177 A | 6/1995  | Jordan, Jr. et al. | 6,050,340 A | 4/2000  | Scott              |
| 5,435,392 A | 7/1995  | Kennedy            | 6,069,313 A | 5/2000  | Kay                |
| 5,439,051 A | 8/1995  | Kennedy et al.     | 6,076,600 A | 6/2000  | Vick, Jr. et al.   |
|             |         |                    | 6,079,496 A | 6/2000  | Hirth              |
|             |         |                    | 6,085,837 A | 7/2000  | Massinon et al.    |
|             |         |                    | 6,095,247 A | 8/2000  | Streich et al.     |
|             |         |                    | 6,119,783 A | 9/2000  | Parker et al.      |

| (56)                  | References Cited |                    |              |         |                      |  |
|-----------------------|------------------|--------------------|--------------|---------|----------------------|--|
| U.S. PATENT DOCUMENTS |                  |                    |              |         |                      |  |
| 6,126,898 A           | 10/2000          | Butler             | 6,613,383 B1 | 9/2003  | George et al.        |  |
| 6,142,237 A           | 11/2000          | Christmas et al.   | 6,619,400 B2 | 9/2003  | Brunet               |  |
| 6,161,622 A           | 12/2000          | Robb et al.        | 6,630,008 B1 | 10/2003 | Meeks, III et al.    |  |
| 6,167,970 B1          | 1/2001           | Stout et al.       | 6,634,428 B2 | 10/2003 | Krauss et al.        |  |
| 6,170,583 B1          | 1/2001           | Boyce              | 6,662,886 B2 | 12/2003 | Russell              |  |
| 6,171,359 B1          | 1/2001           | Levinski et al.    | 6,675,889 B1 | 1/2004  | Mullins et al.       |  |
| 6,173,779 B1          | 1/2001           | Smith              | 6,699,305 B2 | 3/2004  | Myrick               |  |
| 6,176,323 B1          | 1/2001           | Weirich et al.     | 6,712,153 B2 | 3/2004  | Turley et al.        |  |
| 6,189,616 B1          | 2/2001           | Gano et al.        | 6,712,797 B1 | 3/2004  | Southern, Jr.        |  |
| 6,189,618 B1          | 2/2001           | Beeman et al.      | 6,713,177 B2 | 3/2004  | George et al.        |  |
| 6,213,202 B1          | 4/2001           | Read, Jr.          | 6,715,541 B2 | 4/2004  | Pedersen et al.      |  |
| 6,220,349 B1          | 4/2001           | Vargus et al.      | 6,737,385 B2 | 5/2004  | Todd et al.          |  |
| 6,220,350 B1          | 4/2001           | Brothers et al.    | 6,779,599 B2 | 8/2004  | Mullins et al.       |  |
| 6,220,357 B1          | 4/2001           | Carmichael et al.  | 6,799,638 B2 | 10/2004 | Butterfield, Jr.     |  |
| 6,228,904 B1          | 5/2001           | Yadav et al.       | 6,810,960 B2 | 11/2004 | Pia                  |  |
| 6,230,799 B1          | 5/2001           | Slaughter et al.   | 6,817,414 B2 | 11/2004 | Lee                  |  |
| 6,237,688 B1          | 5/2001           | Burleson et al.    | 6,831,044 B2 | 12/2004 | Constien             |  |
| 6,238,280 B1          | 5/2001           | Ritt et al.        | 6,883,611 B2 | 4/2005  | Smith et al.         |  |
| 6,241,021 B1          | 6/2001           | Bowling            | 6,887,297 B2 | 5/2005  | Winter et al.        |  |
| 6,248,399 B1          | 6/2001           | Hehmann            | 6,896,049 B2 | 5/2005  | Moyes                |  |
| 6,250,392 B1          | 6/2001           | Muth               | 6,896,061 B2 | 5/2005  | Hriscu et al.        |  |
| 6,261,432 B1          | 7/2001           | Huber et al.       | 6,899,777 B2 | 5/2005  | Vaidyanathan et al.  |  |
| 6,265,205 B1          | 7/2001           | Hitchens et al.    | 6,908,516 B2 | 6/2005  | Hehmann et al.       |  |
| 6,273,187 B1          | 8/2001           | Voisin, Jr. et al. | 6,913,827 B2 | 7/2005  | George et al.        |  |
| 6,276,452 B1          | 8/2001           | Davis et al.       | 6,926,086 B2 | 8/2005  | Patterson et al.     |  |
| 6,276,457 B1          | 8/2001           | Moffatt et al.     | 6,932,159 B2 | 8/2005  | Hovem                |  |
| 6,279,656 B1          | 8/2001           | Sinclair et al.    | 6,939,388 B2 | 9/2005  | Angeliu              |  |
| 6,287,332 B1          | 9/2001           | Bolz et al.        | 6,945,331 B2 | 9/2005  | Patel                |  |
| 6,287,445 B1          | 9/2001           | Lashmore et al.    | 6,951,331 B2 | 10/2005 | Haughom et al.       |  |
| 6,302,205 B1          | 10/2001          | Ryll               | 6,959,759 B2 | 11/2005 | Doane et al.         |  |
| 6,315,041 B1          | 11/2001          | Carlisle et al.    | 6,973,970 B2 | 12/2005 | Johnston et al.      |  |
| 6,315,050 B2          | 11/2001          | VayInshteyn et al. | 6,973,973 B2 | 12/2005 | Howard et al.        |  |
| 6,325,148 B1          | 12/2001          | Trahan et al.      | 6,983,796 B2 | 1/2006  | Bayne et al.         |  |
| 6,328,110 B1          | 12/2001          | Joubert            | 6,986,390 B2 | 1/2006  | Doane et al.         |  |
| 6,341,653 B1          | 1/2002           | Fermaniuk et al.   | 7,013,989 B2 | 3/2006  | Hammond et al.       |  |
| 6,341,747 B1          | 1/2002           | Schmidt et al.     | 7,013,998 B2 | 3/2006  | Ray et al.           |  |
| 6,349,766 B1          | 2/2002           | Bussear et al.     | 7,017,664 B2 | 3/2006  | Walker et al.        |  |
| 6,354,372 B1          | 3/2002           | Carisell et al.    | 7,017,677 B2 | 3/2006  | Keshavan et al.      |  |
| 6,354,379 B2          | 3/2002           | Miszewski et al.   | 7,021,389 B2 | 4/2006  | Bishop et al.        |  |
| 6,371,206 B1          | 4/2002           | Mills              | 7,025,146 B2 | 4/2006  | King et al.          |  |
| 6,372,346 B1          | 4/2002           | Toth               | 7,028,778 B2 | 4/2006  | Krywitsky            |  |
| 6,382,244 B2          | 5/2002           | Vann               | 7,044,230 B2 | 5/2006  | Starr et al.         |  |
| 6,390,195 B1          | 5/2002           | Nguyen et al.      | 7,048,812 B2 | 5/2006  | Bettles et al.       |  |
| 6,390,200 B1          | 5/2002           | Allamon et al.     | 7,049,272 B2 | 5/2006  | Sinclair et al.      |  |
| 6,394,180 B1          | 5/2002           | Berscheidt et al.  | 7,051,805 B2 | 5/2006  | Doane et al.         |  |
| 6,394,185 B1          | 5/2002           | Constien           | 7,059,410 B2 | 6/2006  | Bousche et al.       |  |
| 6,395,402 B1          | 5/2002           | Lambert et al.     | 7,063,748 B2 | 6/2006  | Talton               |  |
| 6,397,950 B1          | 6/2002           | Streich et al.     | 7,090,027 B1 | 8/2006  | Williams             |  |
| 6,401,547 B1          | 6/2002           | Hatfield et al.    | 7,093,664 B2 | 8/2006  | Todd et al.          |  |
| 6,403,210 B1          | 6/2002           | Stuivinga et al.   | 7,096,945 B2 | 8/2006  | Richards et al.      |  |
| 6,408,946 B1          | 6/2002           | Marshall et al.    | 7,096,946 B2 | 8/2006  | Jasser et al.        |  |
| 6,419,023 B1          | 7/2002           | George et al.      | 7,097,807 B1 | 8/2006  | Meeks, III et al.    |  |
| 6,422,314 B1          | 7/2002           | Todd et al.        | 7,097,906 B2 | 8/2006  | Gardner              |  |
| 6,439,313 B1          | 8/2002           | Thomeer et al.     | 7,108,080 B2 | 9/2006  | Tessari et al.       |  |
| 6,444,316 B1          | 9/2002           | Reddy et al.       | 7,111,682 B2 | 9/2006  | Blaisdell            |  |
| 6,446,717 B1          | 9/2002           | White et al.       | 7,128,145 B2 | 10/2006 | Mickey               |  |
| 6,457,525 B1          | 10/2002          | Scott              | 7,141,207 B2 | 11/2006 | Jandeska, Jr. et al. |  |
| 6,467,546 B2          | 10/2002          | Allamon et al.     | 7,150,326 B2 | 12/2006 | Bishop et al.        |  |
| 6,470,965 B1          | 10/2002          | Winzer             | 7,163,066 B2 | 1/2007  | Lehr                 |  |
| 6,491,097 B1          | 12/2002          | Oneal et al.       | 7,165,622 B2 | 1/2007  | Hirth et al.         |  |
| 6,491,116 B2          | 12/2002          | Berscheidt et al.  | 7,168,494 B2 | 1/2007  | Starr et al.         |  |
| 6,513,598 B2          | 2/2003           | Moore et al.       | 7,174,963 B2 | 2/2007  | Bertelsen            |  |
| 6,513,600 B2          | 2/2003           | Ross               | 7,182,135 B2 | 2/2007  | Szarka               |  |
| 6,527,051 B1          | 3/2003           | Reddy et al.       | 7,188,559 B1 | 3/2007  | Vecchio              |  |
| 6,540,033 B1          | 4/2003           | Sullivan et al.    | 7,210,527 B2 | 5/2007  | Walker et al.        |  |
| 6,543,543 B2          | 4/2003           | Muth               | 7,210,533 B2 | 5/2007  | Starr et al.         |  |
| 6,554,071 B1          | 4/2003           | Reddy et al.       | 7,217,311 B2 | 5/2007  | Hong et al.          |  |
| 6,561,275 B2          | 5/2003           | Glass et al.       | 7,234,530 B2 | 6/2007  | Gass                 |  |
| 6,581,681 B1          | 6/2003           | Zimmerman et al.   | 7,250,188 B2 | 7/2007  | Dodelet et al.       |  |
| 6,588,507 B2          | 7/2003           | Dusterhoff et al.  | 7,252,162 B2 | 8/2007  | Akinlade et al.      |  |
| 6,591,915 B2          | 7/2003           | Burris et al.      | 7,255,172 B2 | 8/2007  | Johnson              |  |
| 6,601,648 B2          | 8/2003           | Ebinger            | 7,255,178 B2 | 8/2007  | Slup et al.          |  |
| 6,601,650 B2          | 8/2003           | Sundararajan       | 7,264,060 B2 | 9/2007  | Wills                |  |
| 6,609,569 B2          | 8/2003           | Howlett et al.     | 7,267,172 B2 | 9/2007  | Hofman               |  |
| 6,612,826 B1          | 9/2003           | Bauer et al.       | 7,267,178 B2 | 9/2007  | Krywitsky            |  |
|                       |                  |                    | 7,270,186 B2 | 9/2007  | Johnson              |  |
|                       |                  |                    | 7,287,592 B2 | 10/2007 | Surjaatmadja et al.  |  |
|                       |                  |                    | 7,311,152 B2 | 12/2007 | Howard et al.        |  |
|                       |                  |                    | 7,316,274 B2 | 1/2008  | Xu et al.            |  |

| (56)                  | References Cited                |              |                            |  |  |
|-----------------------|---------------------------------|--------------|----------------------------|--|--|
| U.S. PATENT DOCUMENTS |                                 |              |                            |  |  |
| 7,320,365 B2          | 1/2008 Pia                      | 7,752,971 B2 | 7/2010 Loehr               |  |  |
| 7,322,412 B2          | 1/2008 Badalamenti et al.       | 7,757,773 B2 | 7/2010 Rytlewski           |  |  |
| 7,322,417 B2          | 1/2008 Rytlewski et al.         | 7,762,342 B2 | 7/2010 Richard et al.      |  |  |
| 7,325,617 B2          | 2/2008 Murray                   | 7,770,652 B2 | 8/2010 Barnett             |  |  |
| 7,328,750 B2          | 2/2008 Swor et al.              | 7,771,289 B2 | 8/2010 Palumbo et al.      |  |  |
| 7,331,388 B2          | 2/2008 Vilela et al.            | 7,771,547 B2 | 8/2010 Biehler et al.      |  |  |
| 7,337,854 B2          | 3/2008 Horn et al.              | 7,775,284 B2 | 8/2010 Richard et al.      |  |  |
| 7,346,456 B2          | 3/2008 Le Bemadjiel             | 7,775,285 B2 | 8/2010 Surjaatmadja et al. |  |  |
| 7,350,582 B2          | 4/2008 McKeachnie et al.        | 7,775,286 B2 | 8/2010 Duphorne            |  |  |
| 7,353,867 B2          | 4/2008 Carter et al.            | 7,784,543 B2 | 8/2010 Johnson             |  |  |
| 7,353,879 B2          | 4/2008 Todd et al.              | 7,793,714 B2 | 9/2010 Johnson             |  |  |
| 7,360,593 B2          | 4/2008 Constien                 | 7,793,820 B2 | 9/2010 Hirano et al.       |  |  |
| 7,360,597 B2          | 4/2008 Blaisdell                | 7,794,520 B2 | 9/2010 Murty et al.        |  |  |
| 7,363,970 B2          | 4/2008 Corre et al.             | 7,798,225 B2 | 9/2010 Giroux et al.       |  |  |
| 7,373,978 B2          | 5/2008 Barry et al.             | 7,798,226 B2 | 9/2010 Themig              |  |  |
| 7,380,600 B2          | 6/2008 Willberg et al.          | 7,798,236 B2 | 9/2010 McKeachnie et al.   |  |  |
| 7,384,443 B2          | 6/2008 Mirchandani              | 7,806,189 B2 | 10/2010 Frazier            |  |  |
| 7,387,158 B2          | 6/2008 Murray et al.            | 7,806,192 B2 | 10/2010 Foster et al.      |  |  |
| 7,387,165 B2          | 6/2008 Lopez de Cardenas et al. | 7,810,553 B2 | 10/2010 Cruickshank et al. |  |  |
| 7,392,841 B2          | 7/2008 Murray et al.            | 7,810,567 B2 | 10/2010 Daniels et al.     |  |  |
| 7,401,648 B2          | 7/2008 Richard                  | 7,819,198 B2 | 10/2010 Birckhead et al.   |  |  |
| 7,416,029 B2          | 8/2008 Telfer et al.            | 7,828,055 B2 | 11/2010 Willauer et al.    |  |  |
| 7,422,058 B2          | 9/2008 O'Malley                 | 7,833,944 B2 | 11/2010 Munoz et al.       |  |  |
| 7,426,964 B2          | 9/2008 Lynde et al.             | 7,849,927 B2 | 12/2010 Herrera            |  |  |
| 7,441,596 B2          | 10/2008 Wood et al.             | 7,851,016 B2 | 12/2010 Arbab et al.       |  |  |
| 7,445,049 B2          | 11/2008 Howard et al.           | 7,855,168 B2 | 12/2010 Fuller et al.      |  |  |
| 7,451,815 B2          | 11/2008 Hailey, Jr.             | 7,861,779 B2 | 1/2011 Vestavik            |  |  |
| 7,451,817 B2          | 11/2008 Reddy et al.            | 7,861,781 B2 | 1/2011 D'Arcy              |  |  |
| 7,461,699 B2          | 12/2008 Richard et al.          | 7,874,365 B2 | 1/2011 East, Jr. et al.    |  |  |
| 7,464,752 B2          | 12/2008 Dale et al.             | 7,878,253 B2 | 2/2011 Stowe et al.        |  |  |
| 7,464,764 B2          | 12/2008 Xu                      | 7,879,162 B2 | 2/2011 Pandey              |  |  |
| 7,472,750 B2          | 1/2009 Walker et al.            | 7,879,367 B2 | 2/2011 Heublein et al.     |  |  |
| 7,478,676 B2          | 1/2009 East, Jr. et al.         | 7,896,091 B2 | 3/2011 Williamson et al.   |  |  |
| 7,491,444 B2          | 2/2009 Smith et al.             | 7,897,063 B1 | 3/2011 Perry et al.        |  |  |
| 7,503,390 B2          | 3/2009 Gomez                    | 7,900,696 B1 | 3/2011 Nish et al.         |  |  |
| 7,503,392 B2          | 3/2009 King et al.              | 7,900,703 B2 | 3/2011 Clark et al.        |  |  |
| 7,503,399 B2          | 3/2009 Badalamenti et al.       | 7,909,096 B2 | 3/2011 Clark et al.        |  |  |
| 7,509,993 B1          | 3/2009 Turng et al.             | 7,909,104 B2 | 3/2011 Bjorgum             |  |  |
| 7,510,018 B2          | 3/2009 Williamson et al.        | 7,909,110 B2 | 3/2011 Sharma et al.       |  |  |
| 7,513,311 B2          | 4/2009 Gramstad et al.          | 7,909,115 B2 | 3/2011 Grove et al.        |  |  |
| 7,516,791 B2          | 4/2009 Bryant et al.            | 7,913,765 B2 | 3/2011 Crow et al.         |  |  |
| 7,520,944 B2          | 4/2009 Johnson                  | 7,918,275 B2 | 4/2011 Clem                |  |  |
| 7,527,103 B2          | 5/2009 Huang et al.             | 7,931,093 B2 | 4/2011 Foster et al.       |  |  |
| 7,531,020 B2          | 5/2009 Woodfield et al.         | 7,938,191 B2 | 5/2011 Vaidya              |  |  |
| 7,531,021 B2          | 5/2009 Woodfield et al.         | 7,946,335 B2 | 5/2011 Bewlay et al.       |  |  |
| 7,537,825 B1          | 5/2009 Wardle et al.            | 7,946,340 B2 | 5/2011 Surjattmadja et al. |  |  |
| 7,552,777 B2          | 6/2009 Murray et al.            | 7,958,940 B2 | 6/2011 Jameson             |  |  |
| 7,552,779 B2          | 6/2009 Murray                   | 7,963,331 B2 | 6/2011 Surjattmadja et al. |  |  |
| 7,559,357 B2          | 7/2009 Clem                     | 7,963,340 B2 | 6/2011 Gramstad et al.     |  |  |
| 7,575,062 B2          | 8/2009 East, Jr.                | 7,963,342 B2 | 6/2011 George              |  |  |
| 7,579,087 B2          | 8/2009 Maloney et al.           | 7,980,300 B2 | 7/2011 Roberts et al.      |  |  |
| 7,591,318 B2          | 9/2009 Tilghman                 | 7,987,906 B1 | 8/2011 Troy                |  |  |
| 7,600,572 B2          | 10/2009 Slup et al.             | 7,992,763 B2 | 8/2011 Vecchio et al.      |  |  |
| 7,604,049 B2          | 10/2009 Vaidya et al.           | 7,999,987 B2 | 8/2011 Dellingler et al.   |  |  |
| 7,604,055 B2          | 10/2009 Richard et al.          | 8,002,821 B2 | 8/2011 Stinson             |  |  |
| 7,607,476 B2          | 10/2009 Tom et al.              | 8,020,619 B1 | 9/2011 Robertson et al.    |  |  |
| 7,617,871 B2          | 11/2009 Surjaatmadja et al.     | 8,020,620 B2 | 9/2011 Daniels et al.      |  |  |
| 7,635,023 B2          | 12/2009 Goldberg et al.         | 8,025,104 B2 | 9/2011 Cooke, Jr.          |  |  |
| 7,640,988 B2          | 1/2010 Phi et al.               | 8,028,767 B2 | 10/2011 Radford et al.     |  |  |
| 7,647,964 B2          | 1/2010 Akbar et al.             | 8,033,331 B2 | 10/2011 Themig             |  |  |
| 7,661,480 B2          | 2/2010 Al-Anazi                 | 8,034,152 B2 | 10/2011 Westin et al.      |  |  |
| 7,661,481 B2          | 2/2010 Todd et al.              | 8,039,422 B1 | 10/2011 Al-Zahrani         |  |  |
| 7,665,537 B2          | 2/2010 Patel et al.             | 8,056,628 B2 | 11/2011 Whitsitt et al.    |  |  |
| 7,686,082 B2          | 3/2010 Marsh                    | 8,056,638 B2 | 11/2011 Clayton et al.     |  |  |
| 7,690,436 B2          | 4/2010 Turley et al.            | 8,109,340 B2 | 2/2012 Doane et al.        |  |  |
| 7,699,101 B2          | 4/2010 Fripp et al.             | 8,114,148 B2 | 2/2012 Atanasoska et al.   |  |  |
| 7,700,038 B2          | 4/2010 Soran et al.             | 8,119,713 B2 | 2/2012 Dubois et al.       |  |  |
| 7,703,511 B2          | 4/2010 Buyers et al.            | 8,127,856 B1 | 3/2012 Nish et al.         |  |  |
| 7,708,078 B2          | 5/2010 Stoesz                   | 8,153,052 B2 | 4/2012 Jackson et al.      |  |  |
| 7,709,421 B2          | 5/2010 Jones et al.             | 8,163,060 B2 | 4/2012 Imanishi et al.     |  |  |
| 7,712,541 B2          | 5/2010 Loretz et al.            | 8,167,043 B2 | 5/2012 Willberg et al.     |  |  |
| 7,723,272 B2          | 5/2010 Crews et al.             | 8,211,247 B2 | 7/2012 Marya et al.        |  |  |
| 7,726,406 B2          | 6/2010 Xu                       | 8,211,248 B2 | 7/2012 Marya               |  |  |
| 7,735,578 B2          | 6/2010 Loehr et al.             | 8,211,331 B2 | 7/2012 Jorgensen et al.    |  |  |
| 7,743,836 B2          | 6/2010 Cook et al.              | 8,220,554 B2 | 7/2012 Jordan et al.       |  |  |
|                       |                                 | 8,226,740 B2 | 7/2012 Chaumonnot et al.   |  |  |
|                       |                                 | 8,230,731 B2 | 7/2012 Dyer et al.         |  |  |
|                       |                                 | 8,231,947 B2 | 7/2012 Vaidya et al.       |  |  |
|                       |                                 | 8,263,178 B2 | 9/2012 Boulos et al.       |  |  |

| (56)                  | References Cited |                      |                 |         |                        |       |
|-----------------------|------------------|----------------------|-----------------|---------|------------------------|-------|
| U.S. PATENT DOCUMENTS |                  |                      |                 |         |                        |       |
| 8,267,177 B1          | 9/2012           | Vogel et al.         | 9,309,733 B2    | 4/2016  | Xu et al.              |       |
| 8,276,670 B2          | 10/2012          | Patel                | 9,309,744 B2    | 4/2016  | Frazier                |       |
| 8,277,974 B2          | 10/2012          | Kumar et al.         | 9,366,106 B2    | 6/2016  | Xu et al.              |       |
| 8,297,364 B2          | 10/2012          | Agrawal et al.       | 9,447,482 B2    | 9/2016  | Kim et al.             |       |
| 8,327,931 B2          | 12/2012          | Agrawal et al.       | 9,458,692 B2    | 10/2016 | Fripp et al.           |       |
| 8,403,037 B2          | 3/2013           | Agrawal et al.       | 9,500,061 B2    | 11/2016 | Frazier et al.         |       |
| 8,413,727 B2          | 4/2013           | Holmes               | 9,528,343 B2    | 12/2016 | Jordan et al.          |       |
| 8,425,651 B2          | 4/2013           | Xu et al.            | 9,587,156 B2    | 3/2017  | Crews                  |       |
| 8,459,347 B2          | 6/2013           | Stout                | 9,605,508 B2    | 3/2017  | Xu                     |       |
| RE44,385 E            | 7/2013           | Johnson              | 9,643,250 B2    | 5/2017  | Mazyar et al.          |       |
| 8,485,265 B2          | 7/2013           | Marya et al.         | 9,682,425 B2    | 6/2017  | Ku et al.              |       |
| 8,486,329 B2          | 7/2013           | Shikai et al.        | 9,689,227 B2    | 6/2017  | Fripp et al.           |       |
| 8,490,674 B2          | 7/2013           | Stevens et al.       | 9,689,231 B2    | 6/2017  | Fripp et al.           |       |
| 8,490,689 B1          | 7/2013           | McClinton et al.     | 9,789,663 B2    | 10/2017 | Zhang et al.           |       |
| 8,506,733 B2          | 8/2013           | Enami et al.         | 9,790,763 B2    | 10/2017 | Fripp et al.           |       |
| 8,528,633 B2          | 9/2013           | Agrawal et al.       | 9,802,250 B2    | 10/2017 | Xu                     |       |
| 8,535,604 B1          | 9/2013           | Baker et al.         | 9,803,439 B2    | 10/2017 | Xu et al.              |       |
| 8,573,295 B2          | 11/2013          | Johnson et al.       | 9,833,838 B2    | 12/2017 | Mazyar et al.          |       |
| 8,579,023 B1          | 11/2013          | Nish et al.          | 9,835,016 B2    | 12/2017 | Zhang et al.           |       |
| 8,613,789 B2          | 12/2013          | Han et al.           | 9,863,201 B2    | 1/2018  | Fripp et al.           |       |
| 8,631,876 B2          | 1/2014           | Xu et al.            | 9,925,589 B2    | 3/2018  | Xu                     |       |
| 8,663,401 B2          | 3/2014           | Marya et al.         | 9,926,763 B2    | 3/2018  | Mazyar et al.          |       |
| 8,668,762 B2          | 3/2014           | Kim et al.           | 9,938,451 B2    | 4/2018  | Crews                  |       |
| 8,695,684 B2          | 4/2014           | Chen et al.          | 9,970,249 B2    | 5/2018  | Zhang et al.           |       |
| 8,695,714 B2          | 4/2014           | Xu                   | 10,016,810 B2   | 7/2018  | Salinas et al.         |       |
| 8,714,268 B2          | 5/2014           | Agrawal et al.       | 10,059,092 B2   | 8/2018  | Welch et al.           |       |
| 8,715,339 B2          | 5/2014           | Atanasoska et al.    | 10,059,867 B2   | 8/2018  | Crews                  |       |
| 8,723,564 B2          | 5/2014           | Kim et al.           | 10,081,853 B2   | 9/2018  | Wilks et al.           |       |
| 8,734,564 B2          | 5/2014           | Kim et al.           | 10,082,008 B2   | 9/2018  | Robey et al.           |       |
| 8,734,602 B2          | 5/2014           | Li et al.            | 10,092,953 B2   | 10/2018 | Mazyar et al.          |       |
| 8,746,342 B1          | 6/2014           | Nish et al.          | 10,119,358 B2   | 11/2018 | Walton et al.          |       |
| 8,770,261 B2          | 7/2014           | Marya                | 10,119,359 B2   | 11/2018 | Frazier                |       |
| 8,776,884 B2          | 7/2014           | Xu                   | 10,125,565 B2   | 11/2018 | Fripp et al.           |       |
| 8,789,610 B2          | 7/2014           | Oxford               | 10,167,691 B2   | 1/2019  | Zhang et al.           |       |
| 8,808,423 B2          | 8/2014           | Kim et al.           | 10,174,578 B2   | 1/2019  | Walton et al.          |       |
| 8,852,363 B2          | 10/2014          | Numano et al.        | 10,202,820 B2   | 2/2019  | Xu et al.              |       |
| 8,905,147 B2          | 12/2014          | Fripp et al.         | 10,221,637 B2   | 3/2019  | Xu et al.              |       |
| 8,950,504 B2          | 2/2015           | Xu et al.            | 10,221,641 B2   | 3/2019  | Zhang et al.           |       |
| 8,956,660 B2          | 2/2015           | Launag et al.        | 10,221,642 B2   | 3/2019  | Zhang et al.           |       |
| 8,967,275 B2          | 3/2015           | Crews                | 10,221,643 B2   | 3/2019  | Zhang et al.           |       |
| 8,978,734 B2          | 3/2015           | Stevens              | 10,227,841 B2   | 3/2019  | Fripp et al.           |       |
| 8,991,485 B2          | 3/2015           | Chenault et al.      | 10,253,590 B2   | 4/2019  | Xu et al.              |       |
| 8,998,978 B2          | 4/2015           | Wang                 | 10,266,923 B2   | 4/2019  | Wilks et al.           |       |
| 9,010,416 B2          | 4/2015           | Xu et al.            | 10,316,601 B2   | 6/2019  | Walton et al.          |       |
| 9,010,424 B2          | 4/2015           | Agrawal et al.       | 10,329,643 B2   | 6/2019  | Wilks et al.           |       |
| 9,016,363 B2          | 4/2015           | Xu et al.            | 10,335,855 B2   | 7/2019  | Welch et al.           |       |
| 9,016,384 B2          | 4/2015           | Xu                   | 10,337,086 B2   | 7/2019  | Wilks et al.           |       |
| 9,022,107 B2          | 5/2015           | Agrawal et al.       | 10,344,568 B2   | 7/2019  | Murphree et al.        |       |
| 9,027,655 B2          | 5/2015           | Xu                   | 10,364,630 B2   | 7/2019  | Ku et al.              |       |
| 9,033,041 B2          | 5/2015           | Baihly et al.        | 10,364,631 B2   | 7/2019  | Xu et al.              |       |
| 9,033,060 B2          | 5/2015           | Xu et al.            | 10,364,632 B2   | 7/2019  | Xu et al.              |       |
| 9,044,397 B2          | 6/2015           | Choi et al.          | 10,450,840 B2   | 10/2019 | Xu                     |       |
| 9,057,117 B2          | 6/2015           | Harrison et al.      | 10,472,909 B2   | 11/2019 | Xu et al.              |       |
| 9,057,242 B2          | 6/2015           | Mazyar et al.        | 10,533,392 B2   | 1/2020  | Walton et al.          |       |
| 9,068,428 B2          | 6/2015           | Mazyar et al.        | 10,544,652 B2   | 1/2020  | Fripp et al.           |       |
| 9,079,246 B2          | 7/2015           | Xu et al.            | 10,597,965 B2   | 3/2020  | Allen                  |       |
| 9,080,098 B2          | 7/2015           | Xu et al.            | 10,612,659 B2   | 4/2020  | Xu et al.              |       |
| 9,080,403 B2          | 7/2015           | Xu et al.            | 10,619,438 B2   | 4/2020  | Fripp et al.           |       |
| 9,080,439 B2          | 7/2015           | O'Malley             | 10,619,445 B2   | 4/2020  | Murphree et al.        |       |
| 9,089,408 B2          | 7/2015           | Xu                   | 10,626,695 B2   | 4/2020  | Fripp et al.           |       |
| 9,090,955 B2          | 7/2015           | Xu et al.            | 10,633,947 B2   | 4/2020  | Fripp et al.           |       |
| 9,090,956 B2          | 7/2015           | Xu                   | 10,655,411 B2   | 5/2020  | Fripp et al.           |       |
| 9,101,978 B2          | 8/2015           | Xu                   | 10,669,797 B2   | 6/2020  | Johnson et al.         |       |
| 9,109,429 B2          | 8/2015           | Xu et al.            | 10,724,321 B2   | 7/2020  | Leonard et al.         |       |
| 9,119,906 B2          | 9/2015           | Tomantschager et al. | 10,737,321 B2   | 8/2020  | Xu                     |       |
| 9,127,515 B2          | 9/2015           | Xu et al.            | 10,781,658 B1   | 9/2020  | Kumar et al.           |       |
| 9,163,467 B2          | 10/2015          | Gaudette et al.      | 10,807,355 B2   | 10/2020 | Welch et al.           |       |
| 9,181,088 B2          | 11/2015          | Sibuet et al.        | 11,613,952 B2 * | 3/2023  | Doud ..... E21B 31/002 | 149/7 |
| 9,187,686 B2          | 11/2015          | Crews                | 2002/0020527 A1 | 2/2002  | Kilaas et al.          |       |
| 9,211,586 B1          | 12/2015          | Lavernia et al.      | 2002/0047058 A1 | 4/2002  | Verhoff et al.         |       |
| 9,217,319 B2          | 12/2015          | Frazier et al.       | 2002/0092654 A1 | 7/2002  | Coronado et al.        |       |
| 9,227,243 B2          | 1/2016           | Xu et al.            | 2002/0104616 A1 | 8/2002  | De et al.              |       |
| 9,243,475 B2          | 1/2016           | Xu                   | 2002/0121081 A1 | 9/2002  | Cesaroni et al.        |       |
| 9,260,935 B2          | 2/2016           | Murphree et al.      | 2002/0139541 A1 | 10/2002 | Sheffield et al.       |       |
| 9,284,803 B2          | 3/2016           | Stone et al.         | 2002/0197181 A1 | 12/2002 | Osawa et al.           |       |
|                       |                  |                      | 2003/0019639 A1 | 1/2003  | Mackay                 |       |
|                       |                  |                      | 2003/0060374 A1 | 3/2003  | Cooke, Jr.             |       |

| (56)                  | References Cited |                      |                  |         |                    |            |  |  |
|-----------------------|------------------|----------------------|------------------|---------|--------------------|------------|--|--|
| U.S. PATENT DOCUMENTS |                  |                      |                  |         |                    |            |  |  |
|                       |                  |                      |                  |         |                    |            |  |  |
| 2003/0104147 A1       | 6/2003           | Bretschneider et al. | 2007/0221373 A1  | 9/2007  | Murray             |            |  |  |
| 2003/0111728 A1       | 6/2003           | Thai et al.          | 2007/0227745 A1  | 10/2007 | Roberts et al.     |            |  |  |
| 2003/0127013 A1       | 7/2003           | Zavitsanos et al.    | 2007/0259994 A1  | 11/2007 | Tour et al.        |            |  |  |
| 2003/0141060 A1       | 7/2003           | Hailey, Jr. et al.   | 2007/0270942 A1  | 11/2007 | Thomas             |            |  |  |
| 2003/0150614 A1       | 8/2003           | Brown et al.         | 2007/0284112 A1  | 12/2007 | Magne et al.       |            |  |  |
| 2003/0155114 A1       | 8/2003           | Pedersen et al.      | 2007/0299510 A1  | 12/2007 | Venkatraman et al. |            |  |  |
| 2003/0173005 A1       | 9/2003           | Higashi              | 2008/0011473 A1  | 1/2008  | Wood et al.        |            |  |  |
| 2004/0005483 A1       | 1/2004           | Lin                  | 2008/0020923 A1  | 1/2008  | Debe et al.        |            |  |  |
| 2004/0055758 A1       | 3/2004           | Brezinski et al.     | 2008/0041500 A1  | 2/2008  | Bronfin            |            |  |  |
| 2004/0069502 A1       | 4/2004           | Luke                 | 2008/0047707 A1  | 2/2008  | Boney et al.       |            |  |  |
| 2004/0089449 A1       | 5/2004           | Walton et al.        | 2008/0060810 A9  | 3/2008  | Nguyen et al.      |            |  |  |
| 2004/0094297 A1       | 5/2004           | Malone et al.        | 2008/0081866 A1  | 4/2008  | Gong et al.        |            |  |  |
| 2004/0154806 A1       | 8/2004           | Bode et al.          | 2008/0093073 A1  | 4/2008  | Bustos et al.      |            |  |  |
| 2004/0159446 A1       | 8/2004           | Haugen et al.        | 2008/0105438 A1* | 5/2008  | Jordan .....       | E21B 7/061 |  |  |
| 2004/0216868 A1       | 11/2004          | Owens, Sr.           |                  |         |                    | 166/117.6  |  |  |
| 2004/0231845 A1       | 11/2004          | Cooke, Jr.           | 2008/0121436 A1  | 5/2008  | Slay et al.        |            |  |  |
| 2004/0244968 A1       | 12/2004          | Cook et al.          | 2008/0127475 A1  | 6/2008  | Griffo             |            |  |  |
| 2004/0256109 A1       | 12/2004          | Johnson              | 2008/0149325 A1  | 6/2008  | Crawford           |            |  |  |
| 2004/0261993 A1       | 12/2004          | Nguyen               | 2008/0149345 A1  | 6/2008  | Marya et al.       |            |  |  |
| 2004/0261994 A1       | 12/2004          | Nguyen et al.        | 2008/0149351 A1  | 6/2008  | Marya et al.       |            |  |  |
| 2005/0064247 A1       | 3/2005           | Sane et al.          | 2008/0169130 A1  | 7/2008  | Norman et al.      |            |  |  |
| 2005/0074612 A1       | 4/2005           | Eklund et al.        | 2008/0175744 A1  | 7/2008  | Motegi             |            |  |  |
| 2005/0098313 A1       | 5/2005           | Atkins et al.        | 2008/0179104 A1  | 7/2008  | Zhang et al.       |            |  |  |
| 2005/0102255 A1       | 5/2005           | Bultman              | 2008/0196801 A1  | 8/2008  | Zhao et al.        |            |  |  |
| 2005/0106316 A1       | 5/2005           | Rigney et al.        | 2008/0202764 A1  | 8/2008  | Clayton et al.     |            |  |  |
| 2005/0161212 A1       | 7/2005           | Leismer et al.       | 2008/0202814 A1  | 8/2008  | Lyons et al.       |            |  |  |
| 2005/0165149 A1       | 7/2005           | Chanak et al.        | 2008/0210473 A1  | 9/2008  | Zhang et al.       |            |  |  |
| 2005/0194141 A1       | 9/2005           | Sinclair et al.      | 2008/0216383 A1  | 9/2008  | Pierick et al.     |            |  |  |
| 2005/0235757 A1       | 10/2005          | De Jonge et al.      | 2008/0220991 A1  | 9/2008  | Slay et al.        |            |  |  |
| 2005/0241824 A1       | 11/2005          | Burris, II et al.    | 2008/0223587 A1  | 9/2008  | Cherewykh          |            |  |  |
| 2005/0241825 A1       | 11/2005          | Burris, II et al.    | 2008/0236829 A1  | 10/2008 | Lynde              |            |  |  |
| 2005/0268746 A1       | 12/2005          | Abkowitz et al.      | 2008/0236842 A1  | 10/2008 | Bhavsar et al.     |            |  |  |
| 2005/0269097 A1       | 12/2005          | Towler               | 2008/0248205 A1  | 10/2008 | Blanchet et al.    |            |  |  |
| 2005/0275143 A1       | 12/2005          | Toth                 | 2008/0248413 A1  | 10/2008 | Ishii et al.       |            |  |  |
| 2005/0279427 A1       | 12/2005          | Park et al.          | 2008/0264205 A1  | 10/2008 | Zeng et al.        |            |  |  |
| 2005/0279501 A1       | 12/2005          | Surjaatmadja et al.  | 2008/0264594 A1  | 10/2008 | Lohmueller et al.  |            |  |  |
| 2006/0012087 A1       | 1/2006           | Matsuda et al.       | 2008/0277980 A1  | 11/2008 | Koda et al.        |            |  |  |
| 2006/0013350 A1       | 1/2006           | Akers                | 2008/0282924 A1  | 11/2008 | Saenger et al.     |            |  |  |
| 2006/0057479 A1       | 3/2006           | Niimi et al.         | 2008/0296024 A1  | 12/2008 | Huang et al.       |            |  |  |
| 2006/0102871 A1       | 5/2006           | Wang et al.          | 2008/0302538 A1  | 12/2008 | Hofman             |            |  |  |
| 2006/0108114 A1       | 5/2006           | Johnson              | 2008/0314581 A1  | 12/2008 | Brown              |            |  |  |
| 2006/0110615 A1       | 5/2006           | Karim et al.         | 2008/0314588 A1  | 12/2008 | Langlais et al.    |            |  |  |
| 2006/0113077 A1       | 6/2006           | Willberg et al.      | 2009/0038858 A1  | 2/2009  | Griffo et al.      |            |  |  |
| 2006/0116696 A1       | 6/2006           | Odermatt et al.      | 2009/0044946 A1  | 2/2009  | Shasteen et al.    |            |  |  |
| 2006/0131031 A1       | 6/2006           | McKeachnie           | 2009/0044955 A1  | 2/2009  | King et al.        |            |  |  |
| 2006/0131081 A1       | 6/2006           | Mirchandani et al.   | 2009/0050334 A1  | 2/2009  | Marya et al.       |            |  |  |
| 2006/0144515 A1       | 7/2006           | Tada et al.          | 2009/0055694 A1  | 3/2009  | Xu                 |            |  |  |
| 2006/0150770 A1       | 7/2006           | Freim, III et al.    | 2009/0065216 A1  | 3/2009  | Frazier            |            |  |  |
| 2006/0153728 A1       | 7/2006           | Schoenung et al.     | 2009/0068051 A1  | 3/2009  | Gross              |            |  |  |
| 2006/0169453 A1       | 8/2006           | Savery et al.        | 2009/0074603 A1  | 3/2009  | Chan et al.        |            |  |  |
| 2006/0175059 A1       | 8/2006           | Sinclair et al.      | 2009/0084600 A1  | 4/2009  | Severance          |            |  |  |
| 2006/0186602 A1       | 8/2006           | Martin et al.        | 2009/0090440 A1  | 4/2009  | Kellett            |            |  |  |
| 2006/0207387 A1       | 9/2006           | Soran et al.         | 2009/0107684 A1  | 4/2009  | Cooke, Jr.         |            |  |  |
| 2006/0269437 A1       | 11/2006          | Pandey               | 2009/0114381 A1  | 5/2009  | Stroobants         |            |  |  |
| 2006/0278405 A1       | 12/2006          | Turley               | 2009/0116992 A1  | 5/2009  | Lee                |            |  |  |
| 2006/0283592 A1       | 12/2006          | Sierra et al.        | 2009/0126436 A1  | 5/2009  | Fly et al.         |            |  |  |
| 2007/0017675 A1       | 1/2007           | Hammami et al.       | 2009/0151949 A1  | 6/2009  | Marya et al.       |            |  |  |
| 2007/0134496 A1       | 1/2007           | Katagiri et al.      | 2009/0152009 A1  | 6/2009  | Slay et al.        |            |  |  |
| 2007/0039161 A1       | 2/2007           | Garcia               | 2009/0155616 A1  | 6/2009  | Thamida            |            |  |  |
| 2007/0044958 A1       | 3/2007           | Rytlewski et al.     | 2009/0159289 A1  | 6/2009  | Avant et al.       |            |  |  |
| 2007/0044966 A1       | 3/2007           | Davies et al.        | 2009/0194745 A1  | 8/2009  | Tanaka             |            |  |  |
| 2007/0051521 A1       | 3/2007           | Fike et al.          | 2009/0205841 A1  | 8/2009  | Kluge et al.       |            |  |  |
| 2007/0053785 A1       | 3/2007           | Hetz et al.          | 2009/0211770 A1  | 8/2009  | Nutley et al.      |            |  |  |
| 2007/0054101 A1       | 3/2007           | Sigalas et al.       | 2009/0226340 A1  | 9/2009  | Marya              |            |  |  |
| 2007/0057415 A1       | 3/2007           | Katagiri et al.      | 2009/0226704 A1  | 9/2009  | Kauppinen et al.   |            |  |  |
| 2007/0062644 A1       | 3/2007           | Nakamura et al.      | 2009/0242202 A1  | 10/2009 | Rispler et al.     |            |  |  |
| 2007/0102199 A1       | 5/2007           | Smith et al.         | 2009/0242208 A1  | 10/2009 | Bolding            |            |  |  |
| 2007/0107899 A1       | 5/2007           | Werner et al.        | 2009/0255667 A1  | 10/2009 | Clem et al.        |            |  |  |
| 2007/0108060 A1       | 5/2007           | Park                 | 2009/0255684 A1  | 10/2009 | Bolding            |            |  |  |
| 2007/0131912 A1       | 6/2007           | Simone et al.        | 2009/0255686 A1  | 10/2009 | Richard et al.     |            |  |  |
| 2007/0151009 A1       | 7/2007           | Conrad, III et al.   | 2009/0260817 A1  | 10/2009 | Gambier et al.     |            |  |  |
| 2007/0151769 A1       | 7/2007           | Slutz et al.         | 2009/0266548 A1  | 10/2009 | Olsen et al.       |            |  |  |
| 2007/0181224 A1       | 8/2007           | Marya et al.         | 2009/0272544 A1  | 11/2009 | Giroux et al.      |            |  |  |
| 2007/0187095 A1       | 8/2007           | Walker et al.        | 2009/0283270 A1  | 11/2009 | Langeslag          |            |  |  |
| 2007/0207182 A1       | 9/2007           | Weber et al.         | 2009/0293672 A1  | 12/2009 | Mirchandani et al. |            |  |  |
|                       |                  |                      | 2009/0301730 A1  | 12/2009 | Gweily             |            |  |  |
|                       |                  |                      | 2009/0308588 A1  | 12/2009 | Howell et al.      |            |  |  |
|                       |                  |                      | 2009/0317556 A1  | 12/2009 | Macary             |            |  |  |
|                       |                  |                      | 2009/0317622 A1  | 12/2009 | Huang et al.       |            |  |  |

| (56)                  | References Cited                         |                  |                                            |  |  |  |  |
|-----------------------|------------------------------------------|------------------|--------------------------------------------|--|--|--|--|
| U.S. PATENT DOCUMENTS |                                          |                  |                                            |  |  |  |  |
| 2010/0003536 A1       | 1/2010 Smith et al.                      | 2012/0168152 A1  | 7/2012 Casciaro                            |  |  |  |  |
| 2010/0012385 A1       | 1/2010 Drivdahl et al.                   | 2012/0177905 A1  | 7/2012 Seals et al.                        |  |  |  |  |
| 2010/0015002 A1       | 1/2010 Barrera et al.                    | 2012/0190593 A1  | 7/2012 Soane et al.                        |  |  |  |  |
| 2010/0015469 A1       | 1/2010 Romanowski                        | 2012/0205120 A1  | 8/2012 Howell                              |  |  |  |  |
| 2010/0025255 A1       | 2/2010 Su et al.                         | 2012/0205872 A1  | 8/2012 Reinhardt et al.                    |  |  |  |  |
| 2010/0038076 A1       | 2/2010 Spray et al.                      | 2012/0211239 A1  | 8/2012 Kritzler et al.                     |  |  |  |  |
| 2010/0038595 A1       | 2/2010 Imholt et al.                     | 2012/0234546 A1  | 9/2012 Xu                                  |  |  |  |  |
| 2010/0040180 A1       | 2/2010 Kim et al.                        | 2012/0234547 A1  | 9/2012 O'Malley et al.                     |  |  |  |  |
| 2010/0044041 A1       | 2/2010 Smith et al.                      | 2012/0247765 A1  | 10/2012 Agrawal et al.                     |  |  |  |  |
| 2010/0051278 A1       | 3/2010 Mytopher et al.                   | 2012/0267101 A1  | 10/2012 Cooke, Jr.                         |  |  |  |  |
| 2010/0055492 A1       | 3/2010 Baroum et al.                     | 2012/0269673 A1  | 10/2012 Koo et al.                         |  |  |  |  |
| 2010/0089583 A1       | 3/2010 Xu et al.                         | 2012/0273229 A1* | 11/2012 Xu ..... B22F 7/04<br>427/596      |  |  |  |  |
| 2010/0116495 A1       | 5/2010 Spray                             | 2012/0318513 A1  | 12/2012 Mazyar et al.                      |  |  |  |  |
| 2010/0119405 A1       | 5/2010 Okamoto et al.                    | 2013/0000985 A1  | 1/2013 Agrawal et al.                      |  |  |  |  |
| 2010/0139930 A1       | 6/2010 Patel et al.                      | 2013/0008671 A1  | 1/2013 Booth                               |  |  |  |  |
| 2010/0161031 A1       | 6/2010 Papirov et al.                    | 2013/0017610 A1  | 1/2013 Roberts et al.                      |  |  |  |  |
| 2010/0200230 A1       | 8/2010 East, Jr. et al.                  | 2013/0022816 A1  | 1/2013 Smith et al.                        |  |  |  |  |
| 2010/0236793 A1       | 9/2010 Bjorgum                           | 2013/0029886 A1  | 1/2013 Mazyar et al.                       |  |  |  |  |
| 2010/0236794 A1       | 9/2010 Duan et al.                       | 2013/0032357 A1  | 2/2013 Mazyar et al.                       |  |  |  |  |
| 2010/0243254 A1       | 9/2010 Murphy et al.                     | 2013/0043041 A1  | 2/2013 McCoy et al.                        |  |  |  |  |
| 2010/0252273 A1       | 10/2010 Duphorne                         | 2013/0047785 A1  | 2/2013 Xu                                  |  |  |  |  |
| 2010/0252280 A1       | 10/2010 Swor et al.                      | 2013/0052472 A1  | 2/2013 Xu                                  |  |  |  |  |
| 2010/0270031 A1       | 10/2010 Patel                            | 2013/0056215 A1  | 3/2013 Crews                               |  |  |  |  |
| 2010/0276136 A1       | 11/2010 Evans et al.                     | 2013/0062049 A1* | 3/2013 Ren ..... B29C 44/5636<br>264/45.3  |  |  |  |  |
| 2010/0276159 A1       | 11/2010 Mailand et al.                   | 2013/0068411 A1  | 3/2013 Forde et al.                        |  |  |  |  |
| 2010/0282338 A1       | 11/2010 Gerrard et al.                   | 2013/0068461 A1  | 3/2013 Maerz et al.                        |  |  |  |  |
| 2010/0282469 A1       | 11/2010 Richard et al.                   | 2013/0084643 A1  | 4/2013 Commarie et al.                     |  |  |  |  |
| 2010/0297432 A1       | 11/2010 Sherman et al.                   | 2013/0105159 A1  | 5/2013 Alvarez et al.                      |  |  |  |  |
| 2010/0304178 A1       | 12/2010 Dirscherl                        | 2013/0112429 A1  | 5/2013 Crews                               |  |  |  |  |
| 2010/0304182 A1       | 12/2010 Facchini et al.                  | 2013/0126190 A1  | 5/2013 Mazyar et al.                       |  |  |  |  |
| 2010/0314105 A1       | 12/2010 Rose                             | 2013/0133897 A1  | 5/2013 Bailhly et al.                      |  |  |  |  |
| 2010/0314127 A1       | 12/2010 Swor et al.                      | 2013/0144290 A1  | 6/2013 Schiff et al.                       |  |  |  |  |
| 2010/0319427 A1       | 12/2010 Lohbeck et al.                   | 2013/0146144 A1  | 6/2013 Joseph et al.                       |  |  |  |  |
| 2010/0326650 A1       | 12/2010 Tran et al.                      | 2013/0160992 A1  | 6/2013 Agrawal et al.                      |  |  |  |  |
| 2011/0005773 A1       | 1/2011 Dusterhoft et al.                 | 2013/0167502 A1  | 7/2013 Wilson et al.                       |  |  |  |  |
| 2011/0036592 A1       | 2/2011 Fay                               | 2013/0168257 A1  | 7/2013 Mazyar et al.                       |  |  |  |  |
| 2011/0048743 A1       | 3/2011 Stafford et al.                   | 2013/0186626 A1  | 7/2013 Aitken et al.                       |  |  |  |  |
| 2011/0052805 A1       | 3/2011 Bordere et al.                    | 2013/0199800 A1  | 8/2013 Kellner et al.                      |  |  |  |  |
| 2011/0067872 A1       | 3/2011 Agrawal                           | 2013/0209308 A1  | 8/2013 Mazyar et al.                       |  |  |  |  |
| 2011/0067889 A1       | 3/2011 Marya et al.                      | 2013/0220496 A1  | 8/2013 Inoue et al.                        |  |  |  |  |
| 2011/0091660 A1       | 4/2011 Dirscherl                         | 2013/0240200 A1  | 9/2013 Frazier                             |  |  |  |  |
| 2011/0094406 A1       | 4/2011 Marya et al.                      | 2013/0240203 A1  | 9/2013 Frazier                             |  |  |  |  |
| 2011/0094737 A1*      | 4/2011 Chen ..... C09K 8/52<br>166/305.1 | 2013/0261735 A1  | 10/2013 Pacetti                            |  |  |  |  |
|                       |                                          | 2013/0277044 A1  | 10/2013 King et al.                        |  |  |  |  |
|                       |                                          | 2013/0310961 A1  | 11/2013 Velez                              |  |  |  |  |
|                       |                                          | 2013/048289 A1   | 12/2013 Mazyar                             |  |  |  |  |
|                       |                                          | 2013/0319668 A1  | 12/2013 Tschetter et al.                   |  |  |  |  |
|                       |                                          | 2013/0327540 A1  | 12/2013 Hamid et al.                       |  |  |  |  |
|                       |                                          | 2013/0333899 A1* | 12/2013 Xu ..... E21B 17/1007<br>166/241.1 |  |  |  |  |
| 2011/0135530 A1       | 6/2011 Xu et al.                         | 2014/0018489 A1  | 1/2014 Johnson                             |  |  |  |  |
| 2011/0135805 A1       | 6/2011 Doucet et al.                     | 2014/0020712 A1  | 1/2014 Benson                              |  |  |  |  |
| 2011/0139465 A1       | 6/2011 Tibbles et al.                    | 2014/0027128 A1  | 1/2014 Johnson                             |  |  |  |  |
| 2011/0147014 A1       | 6/2011 Chen et al.                       | 2014/0060834 A1  | 3/2014 Quintero                            |  |  |  |  |
| 2011/0186306 A1       | 8/2011 Marya et al.                      | 2014/0093417 A1  | 4/2014 Liu                                 |  |  |  |  |
| 2011/0192613 A1       | 8/2011 Garcia et al.                     | 2014/0110112 A1  | 4/2014 Jordan, Jr.                         |  |  |  |  |
| 2011/0214881 A1       | 9/2011 Newton et al.                     | 2014/0116711 A1  | 5/2014 Tang                                |  |  |  |  |
| 2011/0221137 A1       | 9/2011 Obi et al.                        | 2014/0124216 A1  | 5/2014 Fripp et al.                        |  |  |  |  |
| 2011/0236249 A1       | 9/2011 Kim et al.                        | 2014/0154341 A1  | 6/2014 Manuel et al.                       |  |  |  |  |
| 2011/0247833 A1       | 10/2011 Todd et al.                      | 2014/0186207 A1  | 7/2014 Bae et al.                          |  |  |  |  |
| 2011/0253387 A1       | 10/2011 Ervin                            | 2014/0190705 A1  | 7/2014 Fripp                               |  |  |  |  |
| 2011/0259610 A1       | 10/2011 Shkurti et al.                   | 2014/0196889 A1  | 7/2014 Jordan et al.                       |  |  |  |  |
| 2011/0277987 A1       | 11/2011 Frazier                          | 2014/0202284 A1  | 7/2014 Kim                                 |  |  |  |  |
| 2011/0277989 A1       | 11/2011 Frazier                          | 2014/0202708 A1  | 7/2014 Jacob et al.                        |  |  |  |  |
| 2011/0277996 A1       | 11/2011 Cullick et al.                   | 2014/0219861 A1  | 8/2014 Han                                 |  |  |  |  |
| 2011/0284232 A1       | 11/2011 Huang                            | 2014/0224477 A1  | 8/2014 Wiese et al.                        |  |  |  |  |
| 2011/0284240 A1       | 11/2011 Chen et al.                      | 2014/0236284 A1  | 8/2014 Stinson                             |  |  |  |  |
| 2011/0284243 A1       | 11/2011 Frazier                          | 2014/0271333 A1  | 9/2014 Kim et al.                          |  |  |  |  |
| 2011/0300403 A1       | 12/2011 Vecchio et al.                   | 2014/0286810 A1  | 9/2014 Marya                               |  |  |  |  |
| 2011/0314881 A1       | 12/2011 Hatcher et al.                   | 2014/0305627 A1  | 10/2014 Manke                              |  |  |  |  |
| 2012/0046732 A1       | 2/2012 Sillekens et al.                  | 2014/0311731 A1  | 10/2014 Smith                              |  |  |  |  |
| 2012/0067426 A1       | 3/2012 Soni et al.                       | 2014/0311752 A1  | 10/2014 Streich et al.                     |  |  |  |  |
| 2012/0080189 A1       | 4/2012 Marya et al.                      | 2014/0360728 A1  | 12/2014 Tashiro et al.                     |  |  |  |  |
| 2012/0090839 A1       | 4/2012 Rudic                             | 2014/0374086 A1  | 12/2014 Agrawal et al.                     |  |  |  |  |
| 2012/0097384 A1       | 4/2012 Valencia et al.                   | 2015/0060085 A1  | 3/2015 Xu                                  |  |  |  |  |
| 2012/0103135 A1       | 5/2012 Xu et al.                         | 2015/0065401 A1  | 3/2015 Xu et al.                           |  |  |  |  |
| 2012/0125642 A1       | 5/2012 Chenault                          | 2015/0102179 A1  | 4/2015 Mchenry                             |  |  |  |  |
| 2012/0130470 A1       | 5/2012 Agnew et al.                      |                  |                                            |  |  |  |  |
| 2012/0145378 A1       | 6/2012 Frazier                           |                  |                                            |  |  |  |  |
| 2012/0145389 A1       | 6/2012 Fitzpatrick, Jr.                  |                  |                                            |  |  |  |  |
| 2012/0156087 A1       | 6/2012 Kawabata                          |                  |                                            |  |  |  |  |

| (56)            | References Cited         |                      | GB | 2095288     | 9/1982  |
|-----------------|--------------------------|----------------------|----|-------------|---------|
|                 | U.S. PATENT DOCUMENTS    |                      | GB | 2529062     | 2/2016  |
| 2015/0184485 A1 | 7/2015                   | Xu et al.            | JP | H10147830   | 6/1998  |
| 2015/0240337 A1 | 8/2015                   | Sherman et al.       | JP | 2000073152  | 3/2000  |
| 2015/0247376 A1 | 9/2015                   | Tolman et al.        | JP | 2000185725  | 7/2000  |
| 2015/0299838 A1 | 10/2015                  | Doud                 | JP | 2002053902  | 2/2002  |
| 2015/0354311 A1 | 12/2015                  | Okura et al.         | JP | 2004154837  | 6/2004  |
| 2016/0024619 A1 | 1/2016                   | Wilks                | JP | 2004225084  | 8/2004  |
| 2016/0128849 A1 | 5/2016                   | Yan et al.           | JP | 2004225765  | 8/2004  |
| 2016/0201425 A1 | 7/2016                   | Walton               | JP | 2005076052  | 3/2005  |
| 2016/0201427 A1 | 7/2016                   | Fripp                | JP | 2008266734  | 11/2008 |
| 2016/0201435 A1 | 7/2016                   | Fripp et al.         | JP | 2008280565  | 11/2008 |
| 2016/0209391 A1 | 7/2016                   | Zhang et al.         | JP | 2009144207  | 7/2009  |
| 2016/0230494 A1 | 8/2016                   | Fripp et al.         | JP | 2010502840  | 1/2010  |
| 2016/0251934 A1 | 9/2016                   | Walton et al.        | JP | 2012197491  | 10/2012 |
| 2016/0258242 A1 | 9/2016                   | Hayter et al.        | KR | 20130023707 | 3/2013  |
| 2016/0265091 A1 | 9/2016                   | Walton et al.        | RU | 2373375     | 7/2006  |
| 2016/0272882 A1 | 9/2016                   | Stray et al.         | WO | 9111587     | 8/1881  |
| 2016/0279709 A1 | 9/2016                   | Xu et al.            | WO | 1990002655  | 3/1990  |
| 2017/0050159 A1 | 2/2017                   | Ku et al.            | WO | 9200961     | 1/1992  |
| 2017/0266923 A1 | 9/2017                   | Guest et al.         | WO | 1992013978  | 8/1992  |
| 2017/0356266 A1 | 12/2017                  | Arackakudiyil et al. | WO | 9857347     | 12/1998 |
| 2018/0010217 A1 | 1/2018                   | Wilks et al.         | WO | 9909227     | 2/1999  |
| 2018/0023359 A1 | 1/2018                   | Xu                   | WO | 1999027146  | 6/1999  |
| 2018/0178289 A1 | 6/2018                   | Xu et al.            | WO | 9947726     | 9/1999  |
| 2018/0187510 A1 | 7/2018                   | Xu et al.            | WO | 2001001087  | 1/2001  |
| 2018/0216431 A1 | 8/2018                   | Walton et al.        | WO | 2004001087  | 12/2003 |
| 2018/0274317 A1 | 9/2018                   | Hall                 | WO | 2004073889  | 9/2004  |
| 2019/0054523 A1 | 2/2019                   | Wolf et al.          | WO | 2005065281  | 7/2005  |
| 2019/0093450 A1 | 3/2019                   | Walton et al.        | WO | 2007044635  | 4/2007  |
| 2019/0203563 A1 | 7/2019                   | Gano et al.          | WO | 2007095376  | 8/2007  |
| 2019/0249510 A1 | 8/2019                   | Deng et al.          | WO | 2008017156  | 2/2008  |
|                 | FOREIGN PATENT DOCUMENTS |                      | WO | 2008034042  | 3/2008  |
|                 |                          |                      | WO | 2008057045  | 5/2008  |
|                 |                          |                      | WO | 2008079485  | 7/2008  |
| CA              | 2886988                  | 10/2015              | WO | 2008079777  | 7/2008  |
| CN              | 1076968                  | 10/1993              | WO | 2008142129  | 11/2008 |
| CN              | 1079234                  | 12/1993              | WO | 2009055354  | 4/2009  |
| CN              | 1255879                  | 6/2000               | WO | 2009079745  | 7/2009  |
| CN              | 1668545                  | 9/2005               | WO | 2009093420  | 7/2009  |
| CN              | 1882759                  | 12/2006              | WO | 2010012184  | 2/2010  |
| CN              | 101050417                | 10/2007              | WO | 2010038016  | 4/2010  |
| CN              | 101351523                | 1/2009               | WO | 2010083826  | 7/2010  |
| CN              | 101381829                | 3/2009               | WO | 2010110505  | 9/2010  |
| CN              | 101392345                | 3/2009               | WO | 2011071902  | 6/2011  |
| CN              | 101454074                | 6/2009               | WO | 2011071907  | 6/2011  |
| CN              | 101457321                | 6/2009               | WO | 2011071910  | 6/2011  |
| CN              | 101605963                | 12/2009              | WO | 2011130063  | 10/2011 |
| CN              | 101720378                | 6/2010               | WO | 2012015567  | 2/2012  |
| CN              | 102517489                | 6/2012               | WO | 2012071449  | 5/2012  |
| CN              | 102796928                | 11/2012              | WO | 2012091984  | 7/2012  |
| CN              | 103343271                | 10/2013              | WO | 2012149007  | 11/2012 |
| CN              | 103602865                | 2/2014               | WO | 2012164236  | 12/2012 |
| CN              | 103898384                | 7/2014               | WO | 2012174101  | 12/2012 |
| CN              | 104004950                | 8/2014               | WO | 2012175665  | 12/2012 |
| CN              | 104152775                | 11/2014              | WO | 2013019410  | 2/2013  |
| CN              | 104480354                | 4/2015               | WO | 2013019421  | 2/2013  |
| CN              | 201532089                | 4/2015               | WO | 2013053057  | 4/2013  |
| CN              | 104651691                | 5/2015               | WO | 2013078031  | 5/2013  |
| CN              | 105779796                | 7/2016               | WO | 2013109287  | 7/2013  |
| CN              | 106086559                | 11/2016              | WO | 2013122712  | 8/2013  |
| EA              | 200600343                | 6/2006               | WO | 2013154634  | 10/2013 |
| EA              | 200870227                | 2/2009               | WO | 2014100141  | 6/2014  |
| EP              | 0033625                  | 8/1981               | WO | 2014113058  | 7/2014  |
| EP              | 0400574                  | 5/1990               | WO | 2014121384  | 8/2014  |
| EP              | 0470599                  | 2/1998               | WO | 2014210283  | 12/2014 |
| EP              | 1006258                  | 1/2000               | WO | 2015127177  | 8/2015  |
| EP              | 1174385                  | 1/2002               | WO | 2015142862  | 9/2015  |
| EP              | 1412175                  | 4/2004               | WO | 2015161171  | 10/2015 |
| EP              | 1493517                  | 1/2005               | WO | 2015171126  | 11/2015 |
| EP              | 1798301                  | 6/2007               | WO | 2015171585  | 11/2015 |
| EP              | 1857570                  | 11/2007              | WO | 216024974   | 2/2016  |
| EP              | 2088217                  | 8/2009               | WO | 2016032490  | 3/2016  |
| GB              | 912956                   | 12/1962              | WO | 2016032493  | 3/2016  |
| GB              | 1046330                  | 10/1966              | WO | 2016032619  | 3/2016  |
| GB              | 1280833                  | 7/1972               | WO | 2016032620  | 3/2016  |
| GB              | 1357065                  | 6/1974               | WO | 2016032621  | 3/2016  |

(56)

## References Cited

## FOREIGN PATENT DOCUMENTS

|    |            |         |
|----|------------|---------|
| WO | 2016032758 | 3/2016  |
| WO | 2016032761 | 3/2016  |
| WO | 2016036371 | 3/2016  |
| WO | 2016085798 | 6/2016  |
| WO | 2016165041 | 10/2016 |
| WO | 2020018110 | 1/2020  |
| WO | 2020109770 | 6/2020  |

## OTHER PUBLICATIONS

- Shimizu et al., "Multi-walled carbon nanotube-reinforced magnesium alloy composites", *Scripta Materialia*, vol. 58, pp. 267-270 (2008).
- Zhan et al., "Single-wall carbon nanotubes as attractive toughening agents in alumina-based nanocomposites", *Nature Materials*, vol. 2, pp. 38-42 (Jan. 2003).
- Curtin et al., "CNT-reinforced ceramics and metals", *Materials Today*, vol. 7, pp. 44-49 (2004).
- Pardo et al., "Corrosion behavior of magnesium/aluminum alloys in 3.5 wt.% NaCl", *Corrosion Science*, vol. 50, pp. 823-834 (2008).
- Song et L., "Influence of microstructure on the corrosion of diecast AZ91D", *Corrosion Science*, vol. 41, pp. 249-273 (1999).
- Watarai, "Trend of Research and Development for Magnesium Alloys—Reducing the Weight of Structural Materials In Motor Vehicles", *Science & Technology Trends, Quarterly Review*, No. 18, pp. 84-97 (Jan. 2006).
- Saravanan et al., "Mechanically Alloyed Carbon Nanotubes (CNT) Reinforced Nanocrystalline AA 4032: Synthesis and Characterization", *Journal of Minerals & Materials Characterization & Engineering*, vol. 9, No. 11, pp. 1027-1035 (2010).
- Tsipas et al., "Effect of high energy ball milling on titanium-hydroxyapatite powders", *Powder Metallurgy*, vol. 46, No. 1 pp. 73-77 (2003).
- Xie et al., "TEM Observation of Interfaces between Particles in Al—Mg Powder Compacts Prepared by Pulse Electric Current Sintering", *Materials Transactions*, vol. 43, No. 9, pp. 2177-2180 (2002).
- Elsayed et al., "Effect of Consolidation and Extrusion Temperatures on Tensile Properties of Hot Extruded ZK61 Magnesium Alloy Gas Atomized Powders via Spark Plasma Sintering", *Transactions of JWRI*, vol. 38, No. 2, pp. 31.
- Shigematsu et al., "Surface treatment of AZ91D magnesium alloy by aluminum diffusion coating", *Journal of Materials Science Letters*, vol. 19, pp. 473-475 (2000).
- Spencer et al., "Fluidized Bed Polymer Particle ALD Process for Producing HDPE/Alumina Nanocomposites", 12th International Conference on Fluidization, vol. RP4 (2007).
- Maisano, "Cryomilling of Aluminum-Based and Magnesium-Based Metal Powders", Thesis, Virginia Tech (Jan. 2006).
- Walters et al., "A Study of Jets from Unsintered-Powder Metal Lined Nonprecision Small-Caliber Shaped Charges", Army Research Laboratory, Aberdeen Proving Group, MC 21005-5066 (Feb. 2001).
- Sigworth et al. "Grain Refinement of Aluminum Castings Alloys" American Foundry Society; Paper 07-67; pp. 5-7 (2007).
- Momentive, "Titanium Diborid Powder" condensed product brochure; retrieved from <https://www.momentive.com/WorkArea/DownloadAsset.aspx?id=27489;> p. 1 (2012).
- Durbin, "Modeling Dissolution in Aluminum Alloys" Dissertation for Georgia Institute of Technology; retrieved from [https://smartech.gatech.edu/bitstream/handle/1853/6873/durbin\\_tracie\\_L\\_200505\\_phd.pdf?](https://smartech.gatech.edu/bitstream/handle/1853/6873/durbin_tracie_L_200505_phd.pdf?) (2005).
- Pegeut et al., "Influence of cold working on the pitting corrosion resistance of stainless steel" *Corrosion Science*, vol. 49, pp. 1933-1948 (2007).
- Elemental Charts from [chemicalelements.com](http://chemicalelements.com); retrieved Jul. 27, 2017.
- Song et al., "Corrosion Mechanisms of Magnesium Alloys" *Advanced Engg Materials*, vol. 1, No. 1 (1999).
- Zhou et al., "Tensile Mechanical Properties and Strengthening Mechanism of Hybrid Carbon Nanotubes . . ." *Journal of Nanomaterials*, 2012; 2012:851862 (doi: 10.1155/2012/851862) Figs. 6 and 7.
- Trojanova et al., "Mechanical and Acoustic Properties of Magnesium Alloys . . ." *Light Metal Alloys Application*, Chapter 8, Published Jun. 11, 2014 (doi: 10.5772/57454) p. 163, para. [0008], [0014-0015]; [0041-0043].
- AZoNano "Silicon Carbide Nanoparticles—Properties, Applications" <http://www.amazon.com/articles.aspx?ArticleD=3396> p. 2, *Physical Properties, Thermal Properties* (May 9, 2013).
- AZoM "Magnesium AZ91D-F Alloy" <http://www.amazon.com/articles.aspx?ArticleD=8670> p. 1, *Chemical Composition*; p. 2 *Physical Properties* (Jul. 31, 2013).
- Elasser et al., "Silicon Carbide Benefits and Advantages . . ." *Proceedings of the IEEE*, 2002; 906(6):969-986 (doi: 10.1109/JPROC.2002.1021562) p. 970, Table 1.
- Lan et al., "Microstructure and Microhardness of SiC Nanoparticles . . ." *Materials Science and Engineering A*; 386:284-290 (2004).
- Casati et al., "Metal Matrix Composites Reinforced by Nanoparticles", vol. 4:65-83 (2014).
- Shaw, "Corrosion Resistance of Magnesium Alloys", *ASM Handbook*, vol. 13A, pp. 602-606 (2003).
- Ye et al., "Review of recent studies in magnesium matrix composites", *Journal of Material Sciences*, vol. 39, pp. 6153-6171 (2004).
- Hassan et al., "Development of a novel magnesium-copper based composite with improved mechanical properties", *Materials Research Bulletin*, vol. 37, pp. 377-389 (2002).
- Ye et al., "Microstructure and tensile properties of Ti6Al4V/AM60B magnesium matrix composite", *Journal of Alloys and Composites*, vol. 402, 00. 162-169 (2005).
- Kumar et al., "Mechanical and Tribological Behavior of Particulars Reinforced Aluminum metal Matrix Composite", *Journal of Minerals & Materials Characterization and Engineering*, vol. 10, pp. 59-91 (2011).
- Majumdar, "Micromechanics of Discontinuously Reinforced MMCs", *Engineering Mechanics and Analysis of Metal-Matrix Composites*, vol. 21, pp. 395-406 (2001).
- Scharf et al., "Corrosion of AX 91 Secondary Magnesium Alloy", *Advanced Engineering Materials*, vol. 7, No. 12, pp. 1134-1142 (2005).
- Hillis et al., "High Purity Magnesium AM60 Alloy: The Critical Contaminant Limits and the Salt Water Corrosion Performance", *SAE Technical Paper Series* (1986).
- Parwar, S.G., *Influence of Microstructure on the Corrosion Behaviour of Magnesium Alloys*, PhD Dissertation, University of Manchester (2011).
- Czerwinski, "Magnesium Injection Molding", *Technology & Engineering*; Springer Science + Media, LLC, pp. 107-108 (Dec. 2007).
- Metals Handbook, Desk Edition, edited by J.R. David, published by ASM International, pp. 559-574 (1988).
- Saravanan et al., "Fabrication and characterization of pure magnesium-30 vol SiCP particle composite", *Material Science and Eng.*, vol. 276, pp. 108-116 (2000).
- Song et al., Texture evolution and mechanical properties of AZ31B magnesium alloy sheets processed by repeated unidirectional bending, *Journal of Alloys and Compounds*, vol. 489, pp. 475-481 (2010).
- Blawert et al., "Magnesium secondary alloys: Alloy design for magnesium alloys with improved tolerance limits against impurities", *Corrosion Science*, vol. 52, No. 7, pp. 2452-2468 (Jul. 1, 2010).
- Wang et al., "Effect of Ni on microstructures and mechanical properties of AZ102 magnesium alloys" *Zhuzao Foundry, Shenyang Zhuzao Yanjiusuo*, vol. 62, No. 1, pp. 315-318 (Jan. 1, 2013).
- Kim et al., "Effect of aluminum on the corrosion characteristics of Mg—4Ni-xAl alloys", *Corrosion*, vol. 59, No. 3, pp. 228-237 (Jan. 1, 2003) (Abstract only).
- Unsworth et al., "A new magnesium alloy system", *Light Metal Age*, vol. 37, No. 7-8., pp. 29-32 (Jan. 1, 1979).
- Geng et al., "Enhanced age-hardening response of Mg—Zn alloys via Co additions", *Scripta Materialia*, vol. 64, No. 6, pp. 506-509 (Mar. 1, 2011).

(56)

**References Cited****OTHER PUBLICATIONS**

- Zhu et al., "Microstructure and mechanical properties of Mg<sub>6</sub>ZnCuO<sub>6</sub>Zr (wt.%) alloys", *Journal of Alloys and Compounds*, vol. 509, No. 8, pp. 3526-3531 (Dec. 22, 2010) (Abstract Only).
- International Search Authority, International Search Report and Written Opinion for PCT/GB2015/052169 (dated Feb. 17, 2016). Search and Examination Report for GB 1413327.6 (dated Jan. 21, 2015).
- Magnesium Elektron Test Report (Mar. 8, 2005).
- New England Fishery Management Counsel, "Fishery Management Plan for American Lobster Amendment 3" (Jul. 1989).
- Emly, E.F., "Principles of Magnesium Technology" Pergamon Press, Oxford (1966).
- Shaw, "Corrosion Resistance of Magnesium Alloys", *ASM Handbook*, vol. 13A, pp. 692-696 (2003).
- Hanawalt et al., "Corrosion studies of magnesium and its alloys", *Metals Technology*, Technical Paper 1353 (1941).
- The American Foundry Society, Magnesium alloys, casting source directory 8208, available at [www.afsinc.org/files/magnes.pdf](http://www.afsinc.org/files/magnes.pdf).
- Rokhlin, "Magnesium alloys containing rare earth metals structure and properties", *Advances in Metallic Alloys*, vol. 3, Taylor & Francis (2003).
- Ghali, "Corrosion Resistance of Aluminum and Magnesium Alloys" pp. 382-389, Wiley Publishing (2010).
- Kim et al., "High Mechanical Strengths of Mg—Ni—Y and Mg—Cu Amorphous Alloys with Significant Supercooled Liquid Region", *Materials Transactions*, vol. 31, No. 11, pp. 929-934 (1990).
- Tekumalla et al., "Mechanical Properties of Magnesium-Rare Earth Alloy Systems", *Metals*, vol. 5, pp. 1-39 (2014).
- Ashby, "Teach Yourself Phase Diagrams and Phase Transformations", Cambridge, 5th Edition, pp. unknown (Mar. 2009).
- Callister, Materials Science and Engineering An Introduction, 6th Edition, New York, pp. unknown (2003).
- Hanson et al. Constitution of Binary Alloys, McGraw-Hill Book Co. Inc., pp. unknown (1958).
- MSE 2090: Introduction to Materials Science, Chapter 9, pp. unknown (date unknown).
- Metals Handbook, "Metallography, Structures and Phase Diagrams", Aluminum-Magnesium, American Society For Metals, 8th Edition, vol. 8, pp. unknown (1973).
- Metals Handbook, "Metallography, Structures and Phase Diagrams", Magnesium-Nickel, American Society For Metals, 8th Edition, vol. 8, pp. unknown (1973).
- Principles and Prevention of Corrosion, "Volts versus saturated calomel reference electrode", D.A. Jones, p. 170 (1996).
- Medlin, "Mass Balance", handwritten notes (Nov. 2020).
- Metals Handbook, "Metallography, Structures and Phase Diagrams", Aluminum-Iron, American Society For Metals, 8th Edition, vol. 8, p. 260 (1973).
- Metals Handbook, "Metallography, Structures and Phase Diagrams", Aluminum-Nickel, American Society For Metals, 8th Edition, vol. 8, p. 261 (1973).
- Metals Handbook, "Metallography, Structures and Phase Diagrams", Aluminum-Copper, American Society For Metals, 8th Edition, vol. 8, p. 259 (1973).
- Metals Handbook, "Metallography, Structures and Phase Diagrams", Silver-Aluminum, American Society For Metals, 8th Edition, vol. 8, p. 252 (1973).
- Medlin, Declaration of Dona J. Medlin Ph.D., P.E., FASM Under 37 CFR Section 1.68 in Support of Petition For Inter Partes Review of U.S. Pat. No. 9,903,010 (Sep. 2020).
- Li, Qiang, "Translation Declaration and Translation of China Patent Publication No. 103343271" (Jun. 2020).
- Ho et al., The mechanical behavior of magnesium alloy AZ91 reinforced with fine copper particulates, *Materials Science and Engineering A369*, pp. 302-308 (2004).
- Trojanova et al., "Mechanical and fracture properties of an AZ91 Magnesium alloy reinforced by Si and SiC particles", *Composites Science and Technology*, vol. 69, pp. 2256-2264 (2009).
- Lin et al., "Formation of Magnesium Metal Matrix Composites Al<sub>2</sub>O<sub>3</sub>p/AZ91D and Their Mechanical Properties After Heat Treatment" *Acta Metallurgica Slovaca*, vol. 16, pp. 237-245 (2010).
- United States District Court/Northern District of Ohio/Eastern Division, Memorandum Opinion and Order in related Case 1:19-CV-1611 (issued Mar. 29, 2021).
- United States District Court/Northern District of Ohio/Eastern Division, Second Rebuttal Rule 26 Report of Lee A. Swanger, Ph.D., P.E. in related Case 1:19-CV-1611 (filed Nov. 24, 2020).
- U.S. Patent and Trademark Office, Declaration of Dana J. Medlin in Support of Request for Ex Parte Reexamination of U.S. Pat. No. 10,329,653 (filed Jul. 6, 2021).
- United States District Court/Northern District of Ohio/Eastern Division, Supplemental Declaration of Dana J. Medlin, Ph.D. in Support of Opposition to Terves LLC'S Motion for Preliminary Injunction in related Case 1:19-CV-1611 (filed Oct. 15, 2020).
- United States District Court/Northern District of Ohio/Eastern Division, Declaration of Andrew Sherman in Support of Terves' Preliminary Injunction Motion in related Case 1:19-CV-1611 (filed May 1, 2020).
- National Physical Laboratory, "Bimetallic Corrosion" Crown (C) p. 1-14 (2000).
- United States District Court / Western District of Oklahoma, Case No. 5:21-cv-1115, *Magnesium Machine LLC v. Terves LLC*, Docket Report (Jan. 24, 2023).
- United States District Court/ Northern District of Ohio, Case No. 1:19-cv-1611, *Terves LLC v. Yueyang Aerospace New Materials Co. Ltd.*, Partial Docket Report (Jan. 24, 2023).
- U.S. Court of Appeals / Federal District, *Terves LLC v. Yueyang Aerospace New Materials Co. Ltd.*, Docket Report (Jan. 24, 2023).
- United States District Court / West District of Oklahoma, Case No. 5:21-cv-1115, *Magnesium Machine, LLC v. Terves LLC*, "Complaint for Declaration Judgment of Non-Infringement, Invalidity, and Unenforceability of Patents, Tortious Interference Contract and Prospective Economic Advantage and Unfair Competition" (Nov. 23, 2021).
- United States District Court / Northern District of Ohio, Eastern Division, Case No. 1:19-cv-1611, *Terves LLC v. Yueyang Aerospace New Materials Co. Ltd.*, "Memorandum in Support of Defendants' Motion for Summary Judgment" (Nov. 18, 2021).
- Patent Trial and Appeal Board / Federal District, *Chongqing Yanmei Technology Co., LTD v. Terves LLC*; 'Declaration Under 37 CFR 1.68 of Dr. Juan C. Nava, Ph.D. (filed Jan. 24, 2023).
- Curriculum Vitae of Dr. Juan C. Nava, Ph.D.
- Patent Trial and Appeal Board / Federal District, *Chongqing Yanmei Technology Co., LTD v. Terves LLC*; 'Petition for Inter Partes Review of U.S. Pat. No. 10,689,740" (filed Jan. 24, 2023).

\* cited by examiner



Fig. 1



Fig. 2

## FLUID ACTIVATED DISINTEGRATING METAL SYSTEM

The present invention is a continuation application of Serial No. U.S. application Ser. No. 17/124,723 filed Dec. 17, 2020 (now U.S. Pat. No. 11,613,952), which in turn is a continuation application of Serial No. U.S. application Ser. No. 16/110,550 filed Aug. 23, 2018 (now U.S. Pat. No. 11,365,164), which in turn is a continuation of U.S. application Ser. No. 14/627,189 filed Feb. 20, 2015 (now U.S. Pat. No. 10,150,713), which in turn claims priority on U.S. Provisional Application Ser. No. 61/942,870 filed Feb. 21, 2014 and 62/054,597 filed Sep. 24, 2014, all of which are incorporated herein by reference.

### FIELD OF THE INVENTION

The present invention relates to the formation of disintegrating components and materials that can be stored indefinitely or near indefinitely unless activated. The present invention also relates to the production of a reactive composite having controlled reaction kinetics catalyzed by an external stimulus. The invention further relates to a reactive composite system that is inert unless initiated by a certain temperature, pH, and/or other external stimulus after, which it disintegrates in a controlled and repeatable manner.

### BACKGROUND OF THE INVENTION

Reactive materials, which dissolve or corrode when exposed to acid, salt, or other wellbore conditions, have been proposed for some time. Generally, these consist of materials that are engineered to dissolve or corrode. Dissolving polymers have been disclosed and are also used extensively in the pharmaceutical industry for controlled-release drugs. In addition, reactive metal matrix composites have been proposed for use in disintegrating metallic systems, primarily consisting of magnesium-graphite systems, but also magnesium-calcium and other material systems that do not passivate and hence corrode in a rapid manner when in contact with a cathode material, such as graphite or iron.

While some of these systems have enjoyed modest success in reducing well completion costs, they have significant drawbacks, including limited strength and poor reliability. Ideally, components could be used, stored, and handled for long periods of time prior to use and, once activated, can undergo highly reliable disintegration or some other action.

### SUMMARY OF THE INVENTION

The present invention relates to the formation of disintegrating components and materials that can be stored for long periods of time (e.g., at least a month, at least a year, etc.) unless activated. The present invention also relates to the production of a reactive composite having controlled reaction kinetics that can be catalyzed by an external stimulus. The invention further relates to a reactive composite system that is inert or essentially inert unless initiated by a certain temperature, pH, and/or other external stimulus after which it disintegrates in a controlled and repeatable manner. In one non-limiting application of the present invention, the components of the present invention can be used in the forming of wells used in, but not limited to, the oil and gas fracking industry. During the formation of wells, various metal components used to form the well are left in the well. These components must either be removed from the well or destroyed before the well can be fully and/or properly

operational. The present invention is directed to components that can be used during the well forming operation and, once the component has completed its intended use, the component can be caused to disintegrate and/or fracture, thus sufficiently removing and/or fracturing the component so that the well can be fully and/or properly operational.

In one non-limiting aspect of the present invention relates to a hierarchically-designed component or system that includes a core and a surface which are designed to react and/or activate under different conditions. The core material is designed to have a high reaction rate that disintegrates over a period of 0.001 minutes to 100 hours (e.g., 0.001 min., 0.0011 min., 0.0012 min . . . 99.99998 hours, 99.9999 hours, 100 hours, and all time values and ranges therebetween), and typically 30 minutes to 100 hours when exposed to certain environments (e.g., saltwater, electrolyte solutions, water, air, electromagnetic waves, sound waves, etc.). The core is typically designed to generate heat when exposed to various environments (e.g., saltwater, electrolyte solutions, water, air, electromagnetic waves, sound waves, etc.). The core can be formed of one or more layers. The shape of the core is non-limiting. The core is partially or fully surrounded by one or more surface or protective layers that inhibits or prevents the core from reacting and/or disintegrating until a desired time or event. The one or more surfaces or protective layers are designed to be inert unless exposed to an activation conditions such as, but not limited to, temperature, electromagnetic waves, sound waves, certain chemicals, and/or pH. Once the one or more surface or protective layers are removed and/or breached, the core material is activated to cause it to dissolve, corrode, react, fracture, etc. when exposed to certain surrounding conditions. For example, in a well application, the component is partially or fully submersed in a liquid environment that commonly includes water and/or saltwater/electrolytes. The core can be designed to dissolve, corrode, react, fracture, etc. when exposed to the water and/or to saltwater/electrolytes (e.g., HCl, KCl, CaCl<sub>2</sub>, CaBr<sub>2</sub>, ZnBr<sub>2</sub>, brine solutions) in the well once the one or more surface or protective layers about the core are removed and/or breached, thereby causing the component to dissolve or disintegrate in the well. The one or more surface or protective layers can also or alternatively be used to provide structural strength to the hierarchically-designed component.

In another non-limiting aspect of the present invention, the hierarchically-designed component or system can include one or more outer surface or protective layers and a core that is formed of two or more layers. Each layer can have a different function in the component or system; however, this is not required. In one non-limiting configuration, the component or system can include a surface or protective layer that encapsulates a core which is formed of at least two layers. In such an arrangement, the inner layer of the core can be a syntactic or very low-density core; the layer about the inner core layer can be a disintegrating high-strength functional layer; and the surface or protective layer is one or more layers that function as a surface modification layer and/or treatment which is inert unless activated.

In still another non-limiting aspect of the present invention, there is provided a surface-inhibited multilayer, multifunctional component comprising (a) a primary or core unit which includes one or more selected properties of density, dissolution rate, disintegration rate, reaction rate, strength; (b) a reactive surface layer having a complimentary set of properties of one or more of strength, temperature-dependent solubility, pH solubility, and density; and wherein the

core unit and surface layer create an inhibited system that is relatively inert until exposed to an initial condition, after which it is activated. In one non-limiting embodiment, at least 70 weight percent of the core includes a core material selected from the group consisting of a metal, a metal alloy or a metal composite, typically at least 90 weight percent of the core includes a core material selected from the group consisting of a metal, a metal alloy or a metal composite, more typically at least 95 weight percent of the core includes a core material selected from the group consisting of a metal, a metal alloy or a metal composite, and even more typically 100 weight percent of the core includes a core material selected from the group consisting of a metal, a metal alloy or a metal composite. The core can be a magnesium, magnesium alloy or magnesium composite having a dissolution rate in salt-containing water of 0.1-100 mm/hr (e.g., 0.1 mm/hr, 0.101 mm/hr, 0.102 mm/hr 99.998 mm/hr, 99.999 mm/hr, 100 mm/hr and all dissolution values and ranges therebetween) at 100-300° F. (and all temperature values and ranges therebetween). When the core is formed of magnesium, the core includes at least 99 wt % magnesium, and typically at least 99.5 wt % magnesium. When the core is formed of a magnesium alloy, the magnesium content of the magnesium alloy is at least 30 wt %, typically greater than 50%, and more typically at least about 70%. The metals that can be included in the magnesium alloy can include, but are not limited to, aluminum, calcium, lithium, manganese, rare earth metal, silicon, SiC, yttrium, zirconium and/or zinc. As can be appreciated, the core can be formed of other metals and/or non-metals that react, corrode, dissolve or disintegrate at a rate of 0.1-100 mm/hr at 100-300° F. in water or salt water. Non-limiting examples of metals or metal alloys other than magnesium that can be used include aluminum alloys (e.g., aluminum alloys including 75+% aluminum and one or more of bismuth, copper, gallium, magnesium, indium, silicon, tin, and/or zinc); calcium; Ca—Mg, Ca—Al; and Ca-Zn. The core can be formulated and/or designed to be relatively insoluble at one temperature (e.g., room temperature: 60-80° F.), but highly soluble above a certain temperature (e.g., 100° F. or greater). Likewise, the core can also or alternatively be formulated and/or designed to be relatively insoluble in a solution having a certain pH (e.g., acidic pH, basic pH, etc.), but highly soluble in a solution having a different pH. When the component includes a surface coating, the surface coating can be designed to be relatively insoluble at a first temperature (e.g., room temperature, etc.), but highly soluble above or below above the first temperature. The surface layer can be formed of a metal coating (e.g., zinc, zinc alloy, etc.) and/or a polymer coating. In one non-limiting example, a surface layer that is relatively insoluble has a dissolution rate of about 0-0.1 mm/day (all dissolution values and ranges therebetween). In another non-limiting example, a surface layer that is highly soluble has a dissolution rate of 0.1 mm/hr or greater (e.g., 0.1 mm/hr 50 mm/hr and all dissolution values and ranges therebetween). Likewise, the surface layer (when used) can also or alternatively be formulated and/or designed to be relatively insoluble in a solution having a certain pH (e.g., acidic pH, basic pH, etc.), but highly soluble in a solution having a different pH. Non-limiting examples of polymers that can be used include ethylene- $\alpha$ -olefin copolymer; linear styrene-isoprene-styrene copolymer; ethylene-butadiene copolymer; styrene-butadiene-styrene copolymer; copolymer having styrene endblocks and ethylene-butadiene or ethylene-butene mid-blocks; copolymer of ethylene and alpha olefin; ethylene-octene copolymer; ethylene-hexene copolymer; ethylene-

butene copolymer; ethylene-pentene copolymer; ethylene-butene copolymer; polyvinyl alcohol (PVA); and/or polyvinyl butyral (PVB). Also or alternatively, when the component includes a surface layer, the surface layer can include a chemistry that enables the surface layer to be an insoluble layer and then become a soluble layer when reacted with one or more compounds. For example, when the surface layer includes PVA, PVB, and/or similar polymers, the surface layer can be modified using a reversible chemical reaction to be insoluble in high-temperature water, acidic water solutions and/or salt water solutions, and which is soluble in high-temperature water, acidic water solutions and salt water solutions when a chemical trigger is applied. The reversible chemical reaction to make the surface layer insoluble can use trimethylsilyl group or similar silicon-containing organic chemicals. The reversible chemical reaction to make the surface layer soluble again can use ammonium fluoride or a similar compound. This non-limiting type of reversible CHchemistry is illustrated below:



As set forth above, PVA, a compound that is soluble in water, can be made insoluble in water by reacting the PVA with trimethylsilyl group or some similar compound to form an insoluble compound in water. This reaction can take place prior to, during, and/or after the PVA (i.e., surface layer) is applied to the core of the component. The core of the component or a portion of the core of the component can be formed of a material (e.g., magnesium, magnesium alloy, etc.) that reacts, corrodes, dissolves, fractures, etc. when exposed to water. The modified surface layer that is insoluble to water protects the core from the water and inhibits or prevents the core from interacting with the water

while the component is being used in the presence of water. Once the function or task of the component is completed, the component can be simply dissolved, corroded, fractured, disintegrated, etc. by exposing the water-insoluble surface layer to ammonium fluoride or a similar compound. Such exposure causes the surface layer to once again become a water-soluble compound. When the component is in the presence of water, the surface layer dissolves and the core is eventually exposed to the water. Upon exposure to water, the core dissolves, corrodes, fractures, disintegrates, etc. thereby causing the component to also dissolve, fracture, corrode, disintegrate, etc. The thickness of the surface layer and/or degree of solubility of the surface layer can be selected to control the rate at which the component dissolves, corrodes, fractures, disintegrates, etc. Likewise, the type of material used for the core and/or structure of the core can be selected to control the rate at which the component dissolves, corrodes, fractures, disintegrates, etc.

In yet another non-limiting aspect of the present invention, the surface layer can optionally be formed of a material that that resists degradation and/or dissolving when exposed to HCl (e.g., 0.1-3M HCl), KCl (e.g., 0.1-3M KCl),  $\text{CaCl}_2$  (e.g., 0.1-3M  $\text{CaCl}_2$ ),  $\text{CaBr}_2$  (e.g., 0.1-3M  $\text{CaBr}_2$ ),  $\text{ZnBr}_2$  (e.g., 0.1-3M  $\text{ZnBr}_2$ ), or brine solutions (1000-300,000 ppm) at a temperature of up to 60° F., but degrades and/or dissolves at a higher temperature of at least 100° F. In one specific surface layer, the surface layer resists HCl, KCl, and/or brine solutions up to 300° F., but degrades when a trigger (e.g., chemical ion source, fluorine ion source, etc.) is introduced to the solution in contact with the coating. One such coating is silicone-based coating (e.g., polymer-based siloxane two-part coating, 2-part epoxy-siloxane coating cured with amino silane, etc.). When the trigger is a fluorine ion source, the source of the fluorine ion can optionally be HF, ammonium fluoride, or other ionic compound where the fluorine ion will appear in a water solution.

In still yet another non-limiting aspect of the present invention, the surface layer can be applied to the core in a variety of ways (gas deposition, sublimation, solvent application, powder coating, plasma spraying, spraying, dipping, brushing, etc.).

In another non-limiting aspect of the present invention, the surface layer can be a polyurethane base system.

In still another non-limiting aspect of the present invention, the surface layer can be colored using dyes for identification of the type of coating, type of core, type of trigger required, and/or type of hierarchically-designed component or system. In one non-limiting coating application process, an electrostatic coating and thermal curing using either a thermoset or thermoplastic polymer coating is used. Such a coating process is known in the industry as a type of "powder coating."

In still yet another non-limiting aspect of the present invention, there is provided a hierarchically-designed component or system in the form of a low-density reactive hierarchically-designed component or system that includes (a) a core having a compression strength above about 5000 psig (e.g., 5000-30,000 psig and all values or ranges therebetween), but having a low density and tensile strength below 30,000 psig (e.g., magnesium composite, aluminum composite, manganese composite, zinc composite, etc.); and (b) a high-strength surface layer that has a higher density and higher strength than the core, but is also reactive (e.g., zinc or zinc alloy composite, etc.) and wherein the core and surface layer are designed to provide a high strength reactive system that also has an overall density of no more than about 5 g/cc (e.g., 0.5-5 g/cc and all values and ranges therebe-

tween) and a tensile strength in the surface layer at least 32 ksi (e.g., 32-90 ksi and all values and ranges therebetween). In one non-limiting configuration, the core has a density of about 0.9-1.4 g/cc. When the core is a magnesium composite, aluminum composite, manganese composite, or a zinc composite, the core can be formed of particles that are connected together by a binder. The core particles can include iron particles, carbon particles, tungsten particles, silicon particles, boron particles, tantalum particles, aluminum particles, zinc particles, iron particles, copper particles, molybdenum particles, silicon particles, ceramic particles, cobalt particles, nickel particles, rhenium particles, SiC particles, etc. (includes oxides and carbides thereof) having an average particle diameter size of about 5 to 50 microns (e.g., 5 microns, 5.01 microns, 5.02 microns . . . 49.98 microns, 49.99 microns, 50 microns) and any value or range therebetween, that are coated with about 0.3 to 3 microns coating thickness (e.g., 0.3 microns, 0.301 microns, 0.302 microns . . . 2.998 microns, 2.999 microns, 3 microns) and any value or range therebetween, of a matrix of magnesium, magnesium alloy, aluminum, aluminum alloy, manganese, manganese alloy, zinc and/or zinc alloy. The magnesium composite, aluminum composite, manganese composite, or zinc composite can be formulated to react when activated by an electrolyte (e.g., HCl, KCl,  $\text{CaCl}_2$ ,  $\text{CaBr}_2$ ,  $\text{ZnBr}_2$ , or brine solutions), heat, etc., with the reactive binder dissolving at a controlled rate. In one non-limiting configuration, the surface layer is a high-strength zinc alloy. In another non-limiting configuration, the core can have a dissolution rate in salt-containing water of 0.1-100 mm/hr at 100-300° F. In another non-limiting configuration, the surface layer can include a fiber-reinforced metal (e.g., steel wire, graphite fiber reinforced magnesium, etc.) to obtain the desired strength of the surface layer.

In another non-limiting aspect of the present invention, there is provided a reactive hierarchically-designed component or system that includes (a) a core having an active material, and a material that is reactive in a fluid; (b) a selectively reactive surface layer that is unreactive in the a first fluid or first fluid conditions, but dissolves or reacts in a second fluid or a condition different from the first fluid condition; and wherein the core is coated with the selectively reactive surface layer, and wherein the core is formed of a different material from the selectively reactive surface layer, and the coating thickness of the selectively reactive surface layer is less than a diameter of the core. The core can include propellant. In one non-limiting configuration, the core includes a water-reactive material such as lithium, sodium, potassium, lithium aluminum hydride, sodium aluminum hydride, potassium aluminum hydride, magnesium aluminum hydride, lithium borohydride, sodium borohydride, calcium borohydride, magnesium hydride, n-Al, borohydride mixed with alanates, metal hydrides, borohydrides, divalent cation alanates, and/or other water-reactive materials. The surface layer is formulated to protect or insulate the core from external environments wherein the core would be reactive to the external environment. In one non-limiting configuration, the coating is insoluble at room temperature, but soluble at a higher temperature. In another or alternative non-limiting configuration, the surface is or includes PVA or PVB. In another and/or alternative non-limiting configuration, the core includes a reactive binder having a metal fuel and/or oxidizer composite which includes one or more of the following metals: magnesium, zirconium, tantalum, titanium, hafnium, calcium, tungsten, molybdenum, chrome, manganese, silicon, germanium and/or aluminum that is mixed with an oxidizer or thermite pair (e.g., fluorinated or

chlorinated polymers such as polytetrafluoroethylene, polyvinylidene difluoride, oxidizers such as bismuth oxide, potassium perchlorate, potassium or silver nitrate, iron oxide, tungsten or molybdenum oxide, and/or intermetallic thermite such as boron, aluminum, or silicon). In another and/or alternative non-limiting configuration, the binder can include an intermetallic reactive material such as iron-aluminum, nickel-aluminum, titanium-boron, and/or other high energy intermetallic couple. In another and/or alternative non-limiting configuration, the binder can include a fuel, oxidizer, and/or a reactive polymeric material. In another and/or alternative non-limiting configuration, the reactive polymeric material can include aluminum-potassium perchlorate-polyvinylidene difluoride and/or tetrafluoroethylene (THV) polymer. The core can be formed by powder metallurgy techniques (e.g., solid state powder sinter-forging, solid state sinter-extrusion, and spark plasma or field assisted sintering in the solid or semi-solid state). The core can alternatively be formed from melt casting, with or without subsequent deformation and heat treatment. The reactive hierarchically-designed component or system can be used to form a variety of structural components (e.g., valve, plug, ball, sleeve, casing etc.) that are designed to corrode/disintegrate or deflagrate under a controlled external stimulus. The reactive hierarchically-designed component or system can be designed to disintegrate over a controlled period of one hour to three weeks (and all values and ranges therebetween), and/or equivalently at a rate of about 0.05-100 mm/hr upon the imparting of a controlled external stimulus of pH, salt content, electrolyte content, electromagnetic waves, sound waves, vibrations, magnetism, pressure, electricity, and/or temperature. The reactive hierarchically-designed component or system can be designed to deflagrate or otherwise combust or react over a certain time period (e.g., one second to 24 hours and all time values or ranges therebetween) upon exposure to an external trigger (e.g., electrical, thermal, magnetic, or hydraulic signal). The trigger can optionally be direct or through a secondary interaction such as, but not limited to, piezoelectric device, breakable capsule, timer, or other intermediate device to convert an external signal to an initiation electrical and/or thermal event. The deflagration of the reactive hierarchically-designed component or system can be utilized to provide thermal energy, clear obstructions, and/or provide local pressure to a location about the hierarchically-designed component or system in a controlled manner. The reaction of the reactive hierarchically-designed component or system can optionally be designed to generate a physical dimensional change, such as swelling (change in density), deformation, bending, and/or shrinkage in the hierarchically-designed component or system during the reaction. In non-limiting application of the reactive hierarchically-designed component or system, composite matrix material and consolidation process used to form the core and/or the complete structure of the hierarchically-designed component or system can be used to enable simultaneous control of compression yield strength and/or control of compressibility modulus for crush and/or extrusion resistance when the hierarchically-designed component or system is contained in an entrapping orifice, and simultaneously also allow for control over the triggering event and the reaction rate of the reactive hierarchically-designed component or system.

In still another non-limiting aspect of the present invention, there is provided a reactive hierarchically-designed component or system that includes a) a core, the core dissolvable, reactive, or combinations thereof in the presence of a fluid environment; and, b) a surface layer that

partially or fully encapsulates the core, and wherein the surface layer has a different composition from the core, and wherein the surface layer forms a protective layer about the core to inhibit or prevent the core from dissolving, reacting, or combinations thereof when the component is exposed to the fluid environment, and wherein the surface layer is non-dissolvable in the fluid environment until the surface layer is exposed to an activation event which thereafter causes the surface layer to controllably dissolve and/or degrade in the fluid environment, and wherein the core 10 dissolving, reacting, or combinations thereof after the surface layer dissolves and exposes the core to the fluid environment. At least 70 weight percent of the core optionally includes one or more core materials selected from the 15 group consisting of a metal, a metal alloy, a metal composite and a metal compound. The core material optionally including one or more metals or compounds selected from the group consisting of aluminum, calcium, lithium, magnesium, potassium, sodium, lithium aluminum hydride, 20 sodium aluminum hydride, potassium aluminum hydride, magnesium aluminum hydride, lithium borohydride, sodium borohydride, calcium borohydride, magnesium hydride, n-Al, borohydride mixed with alanates, metal hydrides, borohydrides, and divalent cation alanates. The fluid environment 25 optionally is a water-containing environment. The activation event optionally includes one or more events selected from the group consisting of a temperature change of the fluid environment, a pH change of the fluid environment, exposure of the surface layer with an activation compound, a change in composition of fluid environment, 30 exposure of the surface layer to an electrical charge, exposure to of the surface layer to certain electromagnetic waves, a change in salt content of the fluid environment, a change in electrolyte content of the fluid environment, exposure of the surface layer to certain sound waves, exposure of the surface layer to certain vibrations, exposure of the surface layer to certain magnetic waves, and exposure of the surface layer to a certain pressure. The core optionally has a dissolution rate in the fluid environment of 0.1 and 100 mm/hr at 35 40 100-300° F. The surface layer is optionally formulated to be relatively insoluble at a first temperature in the fluid environment and highly soluble in the fluid environment at a second temperature. The surface layer is optionally formulated to be relatively insoluble at a first pH in the fluid environment and highly soluble in the fluid environment at a second pH. The surface layer optionally is chemically modified using a reversible chemical reaction to be insoluble 45 in the fluid environment and soluble in the fluid environment when the chemically modified surface layer is exposed to a chemical compound that is a chemical trigger. The surface layer is optionally chemically modified with a silicon-containing compound. The chemical trigger is optionally a fluorine ion source. There is optionally provided a method for forming the reactive hierarchically-designed component or 50 55 system as set forth above. There is optionally a method for forming the reactive hierarchically-designed component or system into a structure that can be used for a) separating hydraulic fracturing systems and zones for oil and gas drilling, b) structural support or component isolation in oil and gas drilling and completion systems, or combinations thereof.

In yet another non-limiting aspect of the present invention, there is provided a reactive hierarchically-designed component or system that includes (a) a core having a compression strength above 5000 psig, a density of no more than 1.7 g/cc and a tensile strength of less than 30,000 psig; 60 (b) a high-strength surface layer that has a greater density

and higher strength than the core, the surface layer partially of fully encapsulating the core; and wherein the core and the surface layer are provide a high-strength reactive system that also has an overall lower density than approximately 4 g/cc and a strength in the surface layer of at least 35 ksi. The core is optionally a magnesium composite or aluminum composite having a density of 0.9-1.4 g/cc. The surface layer is optionally a zinc alloy. The core optionally has a dissolution rate in a salt water environment of 0.1 and 100 mm/hr at 100-300° F. The surface layer optionally includes a fiber-reinforced metal. There is optionally provided a method for forming the reactive hierarchically-designed component or system as set forth above. There is optionally a method for forming the reactive hierarchically-designed component or system into a structure that can be used for a) separating hydraulic fracturing systems and zones for oil and gas drilling, b) structural support or component isolation in oil and gas drilling and completion systems, or combinations thereof.

In still yet another non-limiting aspect of the present invention, there is provided a reactive hierarchically-designed component or system that includes (a) a core that includes an active material that is reactive in a fluid environment; (b) a propellant located in the core, about the core, or combinations thereof; and, (c) a surface layer that partially or fully encapsulates the core, the propellant, or combinations thereof, and wherein the surface layer has a different composition from the core and the propellant, and wherein the propellant has a different composition from the core, and wherein the surface layer forms a protective layer about the core and the propellant to inhibit or prevent the core and the propellant from dissolving, reacting, or combinations thereof when the component is exposed to the fluid environment, and wherein the surface layer is non-dissolvable in the fluid environment until the surface layer is exposed to an activation event which thereafter causes the surface layer to controllably dissolve and/or degrade in the fluid environment and the core and the propellant dissolving, reacting, or combinations thereof after the surface layer dissolves and/or degrades and exposes the core and/or the propellant to the fluid environment. The propellant optionally includes one or more water-reactive material selected from the group consisting of lithium, sodium, potassium, lithium aluminum hydride, sodium aluminum hydride, potassium aluminum hydride, magnesium aluminum hydride, lithium borohydride, sodium borohydride, calcium borohydride, magnesium hydride, n-Al, borohydride mixed with alanates, metal hydrides, borohydrides, divalent cation alanates, and/or other water-reactive materials. The reaction of the propellant with the fluid environment optionally causes rapid heat generation which in turn causes the core to ignite. The fluid environment optionally is a water-containing environment. The activation event optionally includes one or more events selected from the group consisting of a temperature change of the fluid environment, a pH change of the fluid environment, exposure of the surface layer with an activation compound, a change in composition of fluid environment, exposure of the surface layer to an electrical charge, exposure to of the surface layer to certain electromagnetic waves, a change in salt content of the fluid environment, a change in electrolyte content of the fluid environment, exposure of the surface layer to certain sound waves, exposure of the surface layer to certain vibrations, exposure of the surface layer to certain magnetic waves, and exposure of the surface layer to a certain pressure. The surface layer is optionally formulated to be relatively insoluble at a first temperature in the fluid environment and

highly soluble in the fluid environment at a second temperature. The surface layer is optionally formulated to be relatively insoluble at a first pH in the fluid environment and highly soluble in the fluid environment at a second pH. The surface layer is optionally chemically modified using a reversible chemical reaction to be insoluble in the fluid environment and soluble in the fluid environment when the chemically-modified surface layer exposed to a chemical compound that is a chemical trigger. The surface layer 10 optionally is chemically modified with a silicon containing compound. The chemical trigger is optionally a fluorine ion source. The core optionally includes a metal fuel and oxidizer composite which includes one or more mixtures of a reactive metal, an oxidizer, or thermite pair, the reactive metal including one or more metals selected from the group 15 consisting of magnesium, zirconium, tantalum, titanium, hafnium, calcium, tungsten, molybdenum, chrome, manganese, silicon, germanium and aluminum, the oxidizer or thermite pair including one or more compounds selected from the group consisting of fluorinated or chlorinated polymer, oxidizer, and intermetallic thermite. The core 20 optionally includes a binder that includes an intermetallic reactive material that includes a metal material selected from the group consisting of iron-aluminum, nickel-aluminum, titanium-boron, high energy intermetallic couple, or combinations thereof. The binder optionally includes a fuel, an oxidizer, and a reactive polymeric material. The reactive polymeric material optionally includes aluminum-potassium perchlorate-polyvinylidene difluoride or tetrafluoroethylene 25 (THV) polymer. There is optionally provided a method for forming the reactive hierarchically-designed component or system as set forth above. There is optionally a method for forming the reactive hierarchically-designed component or system into a structure that can be used for a) separating hydraulic fracturing systems and zones for oil and gas drilling, b) structural support or component isolation in oil 30 and gas drilling and completion systems, or combinations thereof.

In another non-limiting aspect of the present invention, 40 there is provided a reactive hierarchically-designed component or system that is formed in to structural material that is designed to corrode/disintegrate or deflagrate under a controlled external stimulus. The structural material is optionally designed to disintegrate over a controlled period of one hour to one month or at a rate of about 0.1 to 100 mm/hr upon the imparting of a controlled external stimulus to the structural component. The structural material is optionally 45 designed to deflagrate or otherwise combust or react over a one-second to one-hour period upon an external trigger, and wherein the deflagration is utilized to provide thermal energy, clear obstructions, provide local pressure, or combinations thereof in a controlled manner. The reaction is optionally designed to generate a physical dimensional change, deformation, bending, shrinkage, or combinations 50 thereof.

In one non-limiting object of the present invention, there is provided a component or system that can be controllably disintegrated.

In another and/or alternative non-limiting object of the 60 present invention, there is provided a component or system that can be used in a well operation that can be controllably disintegrated.

In still another and/or alternative non-limiting object of the present invention, there is provided a component or system that can include a core material having a surface or protective layer and which component or system can be stored for long periods of time unless activated.

## 11

In yet another and/or alternative non-limiting object of the present invention, there is provided a component or system that can include a core material having a surface or protective layer and which component or system has controlled reaction kinetics that can be catalyzed by an external stimulus.

In still yet another and/or alternative non-limiting object of the present invention, there is provided a component or system that can include a core material having a surface or protective layer and which component or system has a reactive composite system that is inert or essentially inert unless initiated by a certain temperatures, electromagnetic waves, sound waves, vibrations, chemicals, liquids, gasses, electromagnetic waves, pH, salt content, exposure electrolyte content, magnetism, pressure, and/or exposure to electricity and/or other external stimulus after which it disintegrates in a controlled and repeatable manner.

In another and/or alternative non-limiting object of the present invention, there is provided a component or system that can include a core material having a surface or protective layer and which component or system has a hierarchically-designed component or system that includes a core and a surface which are designed to react and/or activate under different conditions.

In still another and/or alternative non-limiting object of the present invention, there is provided a component or system that can include a core material having a surface or protective layer and which component or system has a core material is designed to have a high reaction rate that disintegrates when exposed to certain environments (liquids, gasses, temperatures, electromagnetic waves, vibrations, and/or sound waves, pH, salt content, electrolyte content, magnetism, pressure, and/or temperature, etc.).

In yet another and/or alternative non-limiting object of the present invention, there is provided a component or system that can include a core material having a surface or protective layer and which component or system has a core material is designed to generate heat when exposed to various environments (e.g., liquids, gasses, temperatures, electromagnetic waves, vibrations, and/or sound waves, pH, salt content, electrolyte content, magnetism, pressure, electricity, and/or temperature, etc.).

In still yet another and/or alternative non-limiting object of the present invention, there is provided a component or system that can include a core material having a surface or protective layer and which component or system has a core material is formed of one or more layers.

In another and/or alternative non-limiting object of the present invention, there is provided a component or system that can include a core material having a surface or protective layer and which component or system has a core material that is partially or fully surrounded by one or more surface or protective layers that inhibits or prevents the core from reacting and/or disintegrating until a desired time or event.

In still another and/or alternative non-limiting object of the present invention, there is provided a component or system that can include a core material having a surface or protective layer and which component or system has one or more surfaces or protective layers that are designed to be inert unless exposed to an activation event or condition, which activation event or condition could be, but are not limited to, temperature, electromagnetic waves, sound waves, certain chemicals, and/or pH.

In yet another and/or alternative non-limiting object of the present invention, there is provided a component or system that can include a core material having a surface or protec-

## 12

tive layer and in which each layer of the component or system has a different function in the component or system.

In still yet another and/or alternative non-limiting object of the present invention, there is provided a component or system that can be used as a dissolvable, degradable and/or reactive structure in oil drilling. For example, the component or system of the present invention can be used to form a frac ball or other structure in a well drilling or completion operation such as a structure that is seated in a hydraulic operation that can be dissolved away after use so that that no drilling or removal of the structure is necessary. Other types of structures can include, but are not limited to, sleeves, valves, hydraulic actuating tooling and the like. Such non-limiting structures or additional non-limiting structure are illustrated in U.S. Pat. Nos. 8,905,147; 8,717,268; 8,663,401; 8,631,876; 8,573,295; 8,528,633; 8,485,265; 8,403,037; 8,413,727; 8,211,331; 7,647,964; US 2013/0199800; US 2013/0032357; US 2013/0029886; US 2007/0181224; and WO 2013/122712; all of which are incorporated herein by reference.

These and other objects, features and advantages of the present invention will become apparent in light of the following detailed description of preferred embodiments thereof, as illustrated in the accompanying drawings.

## BRIEF DESCRIPTION OF THE DRAWINGS

FIGS. 1-2 are a cross-sectional illustration of layered ball actuators in accordance with the present invention wherein the core represents a disintegrating high strength material.

## DETAILED DESCRIPTION OF THE INVENTION

Referring now to the figures wherein the showings illustrate non-limiting embodiments of the present invention, the present invention is directed to the formation and use of disintegrating components and materials that can be stored for long periods of time until activated. The present invention also relates to the production of a reactive hierarchically-designed component or system having controlled reaction kinetics that can be catalyzed by an external stimulus. The invention further relates to a reactive hierarchically-designed component or system that is inert or essentially inert unless initiated by a certain temperature, pH, and/or other external stimulus after which it disintegrates in a controlled and repeatable manner. The components of the present invention have particular applicability to components used in the forming of wells; however, it will be appreciated that the components of the present invention can be used in many other industries and applications.

Referring to FIGS. 1-2, there are cross-sectional illustrations of layered composite ball actuators in accordance with the present invention wherein the core represents a disintegrating high strength composite. The cross-sectional shape of the core illustrated as being circular; however, it can be appreciated that the core can have any shape.

In one non-limiting configuration, the core can be formed of a metal such as, but not limited to, lithium, sodium, magnesium, magnesium-carbon-iron composite system, and the like. As can be appreciated, the core can also or alternatively include a polymer material. The core can be formed of more than one type of material; however, that is not required. The core can be formed of one or more layers. When the core includes two or more layers, the layers are generally formed of different materials; however, this is not required. The surface layer of the composite ball actuator

## 13

can include a protective or delay coating. The surface layer can be a metal layer, a polymer layer, and/or a ceramic layer. The surface layer can be formed of one or more layers. When the surface layer includes two or more layers, the layers are generally formed of different materials; however, this is not required.

In one non-limiting arrangement, the surface layer can be a temperature-sensitive polymer such as, but not limited to, PVA, that is inert and insoluble until exposed to certain environmental conditions. For example, when the surface layer is PVA, and when the PVA reaches a critical temperature in water, the PVA dissolves to expose the underlying reactive core, thereby causing the core to react. Surface layers that activate under exposure to specific temperatures, pressures, fluids, electromagnetic waves and/or mechanical environments to delay the initiation of a dissolution reaction are envisioned by the present invention.

In accordance with the present invention, a metal, metal alloy, metal matrix composite, polymer, or polymer composite having a specified reactive function can form all or part of the core. One of the primary functions of the core is for the material of the core to partially or fully disintegrate in a controlled and uniform manner upon exposure an environmental condition (e.g., exposure to saltwater, etc.). On the surface of the core (which core can be a casting, forging, extrusion, pressed, molded, or machined part), a surface layer is included to modify the conditions to which the core will react. In one non-limiting configuration, the core has a strength above 25,000 psig, and is selected to respond to a set of environmental conditions to perform a function (e.g., react, dissolve, corrode, fracture, generate heat, etc.).

In one non-limiting formulation, the core can be or include magnesium or magnesium alloy that has a temperature-dependent dissolution or disintegration rate. This disintegration rate of the core can be designed such that the core dissolves, corrodes, reacts, and/or chemically reacts in a certain period of time at a given temperature. One non-limiting application that can use such a core is a frac ball. The composite system can be designed such that the core does not disintegrate at a temperature of less than about 100° F. via protection from the surface layer. As can be appreciated, the temperature can be any temperature (e.g., below 10° F., below 50° F., below 100° F., below 150° F., below 200° F., etc.). In one embodiment, wherein the hierarchically-designed component or system is designed to inhibit or prevent reaction of the core at a temperature below 100° F., the core would have a near-infinite life at conditions below 100° F. To accomplish this non-limiting embodiment, the hierarchically-designed component or system has a surface layer that is applied to the surface of the core, wherein the surface layer is inert under conditions wherein the temperature is below 100° F., but dissolves, corrodes, or degrades once the temperature exceeds 100° F. (e.g., dissolves, corrodes, or degrades in the presence of water that exceeds 100° F., dissolves, corrode, or degrades in the present of air that exceeds 100° F., etc.) In this non-limiting embodiment, the kinetics of the reaction can be changed by inhibiting the initial reaction, and then accelerating the reaction once specific conditions are met. As can be appreciated, the surface layer can be caused to dissolve, corrode, or degrade upon exposure to other conditions (e.g., certain liquids, certain gasses, certain temperatures, certain electromagnetic waves, certain vibrations, and/or certain sound waves, certain pH, certain salt content, certain electrolyte content, certain magnetism, certain pressure, electricity, and/or certain temperature, etc.).

## 14

Because the surface layer may be exposed to high stress, surface layer can be thin (e.g., 0.01-50 mils, typically 0.01-10 mils, more typically 0.01-5 mils, etc.); however, this is not required. Alternatively, the surface layer can be designed to be strong and to contribute mechanically to the system, such as through the use of fiber, flakes, metals, metal alloys, and/or whisker reinforcement in the layer. The thickness of the surface layer about the core can be uniform or vary.

10

## Example 1

A magnesium frac ball is produced having a disintegration rate of about 0.7-1.4 mm/hr at 200° F. and about 0.01-0.04 mm/hr at 100° F. The frac ball is designed to be able to withstand at least a 24-hour exposure to 80° F. water in a ball drop system. The magnesium core can be magnesium, magnesium alloy or a magnesium composite. As can be appreciated, the core can be formed of other metals and/or non-metals that react, dissolve, corrode, or disintegrate at a rate of 0.1-100 mm/hr at 100-300° F. in water or salt water. The magnesium frac ball can be undermachined by 0.001-0.2" (e.g., 0.005", etc.) from final dimensions, and a 0.001-0.2" coating (e.g., 0.005" coating, etc.) of PVA can be applied to the surface through a spray-coating process. FIG. 1 illustrates one non-limiting configuration of the frac ball. Although not illustrated in FIG. 1, the core can be formed of multiple layers of material wherein each layer has a different composition from the adjacently positioned layer. For example, the first or central layer of the core could include a magnesium composite material, and a second layer that is applied about the first layer could be magnesium or magnesium alloy. Likewise, the surface layer can include one or more different layers wherein each layer has a different composition from the adjacently positioned layer. The thickness of the two or more layers of the surface layer (when used) can be the same or different. Likewise, the thickness of the two or more layers of the core (when used) can be the same or different. The PVA is very insoluble in water up to about 130-150° F. At temperatures above 150° F., the PVA becomes dissolvable and ultimately exposes the magnesium core. The magnesium frac ball has excellent mechanical properties (e.g., generally above 30 ksi strength), and when the magnesium frac ball is exposed to slightly acidic or salt solutions, the magnesium frac ball corrodes at a rate of about 0.1-15 mm/day. However, when the magnesium frac ball is exposed to temperatures below about 130° F., the magnesium frac ball does not dissolve or corrode. As can be appreciated, the thickness of the coating of PVA can be selected to control the time needed for the PVA to dissolve and thereby expose the core to the surrounding environment.

30

35

40

45

50

55

60

65

## Example 2

A high-strength frac ball is produced using a low-density core, which frac ball is selected for having good compressive strength and low density, and having a surface layer of a higher tensile strength and a denser material than the core. The core is selected from a magnesium composite that uses a high corrosion magnesium alloy matrix with carbon, glass, and/or ceramic microballoons or balls to reduce its density to below 1.7 g/cc (e.g., 0.5-1.66 g/cc and all values and ranges therebetween) and typically below about 1.3 g/cc. As can be appreciated, other densities of the core can be used. This composite core has very good compressive strengths, but tensile strengths may, in some applications, be inadequate for the intended application. For example, the tensile

## 15

strength of the composite core may be less than 35 ksi, typically less than 32 ksi, and more typically less than 30 ksi. As such, the composite core can be surrounded by another layer having a greater tensile strength. This surrounding layer can have a thickness of about 0.035-0.75" (and all values and ranges therebetween) and typically about 0.1-0.2". The surrounding layer can be formed of magnesium, magnesium alloy or a high-strength magnesium composite. The high strength outer layer is designed to have adequate tensile strength and toughness for the applications, and generally has a tensile strength that is greater than 33 ksi, typically greater than 35 ksi, and more typically greater than 45 ksi; however, the tensile strength can have other values. The resultant component can have an overall density of about 5-45% lower (and all values and ranges therebetween) than a pure magnesium alloy ball, and typically about 30% lower than a pure magnesium alloy ball, but also has the high tensile and shear strengths needed to perform the desired ball actuator application.

The core of the high-strength frac ball can be heat treated and machined after fabrication. A surface layer can optionally be applied to the core using thermal spray, co-extrusion, casting, or through power metallurgy techniques suitable for its fabrication as discussed in Example 1.

## Example 3

A magnesium frac ball is produced having a disintegration rate of about 0.7-1.4 mm/hr at 200° F. and about 0.01-0.04 mm/hr at 100° F. The frac ball is designed to be able to withstand at least a 24-hour exposure to 80° F. water in a ball drop system. The magnesium frac ball can be undermachined by 0.001-0.2" (e.g., 0.005", etc.) from final dimensions, and a 0.001-0.2" coating (e.g., 0.005" coating, etc.) of zinc metal can be applied to the surface of the magnesium core. The magnesium core can be magnesium, magnesium alloy or a magnesium composite. As can be appreciated, the core can be formed of other metal and/or non-metals that react, corrode, dissolve or disintegrate at a rate of 0.1-100 mm/hr at 100-300° F. in water or salt water. The resultant compact has high mechanical properties, generally about 28 ksi and typically above 30 ksi strength (e.g., 30-45 ksi and all values and ranges therebetween). When the core of the magnesium frac ball is exposed to salt solutions, the magnesium frac ball corrodes at a rate of about 0.1-15 mm/day depending on the environment and temperature. The magnesium frac ball is designed to not react or corrode until activated with an acid exposure that removes the zinc surface layer and exposes the underlying magnesium core.

## Example 4

A high-strength frac ball is produced using a low-density core, which frac ball is selected for having good compressive strength and low density, and having a surface layer of a higher tensile strength, and a denser material than the core. The core is selected from a magnesium composite that uses a high corrosion magnesium alloy matrix with carbon, glass, and/or ceramic microballoons or balls to reduce its density to below 1.7 g/cc (e.g., 0.5-1.66 g/cc and all values and ranges therebetween) and typically below about 1.3 g/cc. As can be appreciated, other densities of the core can be used. This composite core has very good compressive strengths, but tensile strengths may, in some applications, be inadequate for the intended application. For example, the tensile strength of the composite core may be less than 35 ksi, typically less than 32 ksi, and more typically less than 30 ksi.

## 16

As such, the composite core can be surrounded by another layer having a greater tensile strength. Surrounding the composite core is high-strength metal or metal alloy (e.g., zinc, etc.) that has a layer thickness of about 0.035-0.75", and typically about 0.1-0.2". The high-strength metal or metal alloy outer layer is designed to have adequate tensile strength and toughness for certain the applications, and is generally greater than 33 ksi, typically greater than 35 ksi, and more typically greater than 45 ksi; however, the tensile strength can have other values. The resultant component can have an overall density of about 5-60% lower (and all values and ranges therebetween) than a pure zinc alloy ball, and typically about 50% lower than a pure zinc alloy ball, but also has the high tensile and shear strengths needed to perform the desired ball actuator application.

## Example 5

A reactive material containing a water-reactive substance such as, but not limited to, lithium, is formed into a particle. The lithium is added to a propellant mixture. The propellant mixture can include polyvinylidene difluoride (PVDF), ammonium nitrate, and/or aluminum to form a gas-generating composition. The lithium particle can optionally include a polymer coating (e.g., PVA, etc.) that is applied to its surface to protect it from contact with water. The polymer coating is formulated to be insoluble at room temperature, but can dissolve in hot water (e.g., +140° F.). Once the coating is dissolved to expose the lithium, the lithium reacts with water and releases heat, thus igniting the propellant (e.g., aluminum-ammonium nitrate-PVDF propellant, etc.) to generate heat and gas pressure. As can be appreciated, other reactive particles can be used (e.g., lithium, sodium, potassium, lithium aluminum hydride, sodium aluminum hydride, potassium aluminum hydride, magnesium aluminum hydride, lithium borohydride, sodium borohydride, calcium borohydride, magnesium hydride, n-Al, borohydride mixed with alanates, metal hydrides, borohydrides, divalent cation alanates, and/or other water-reactive materials, etc.).

## Example 6

A reactive material containing a water-reactive substance such as, but not limited to, sodium, is formed into a particle. The sodium is added to a propellant mixture. The propellant mixture can include PVDF, ammonium nitrate, and/or aluminum to form a gas-generating composition. The sodium particle can optionally include a polymer coating (e.g., PVAP, etc.) that is applied to its surface to protect it from contact with water. The polymer can optionally be a polymer that is insoluble in water-containing environments having an acidic pH, but is soluble in neutral or basic water containing environments; however, this is not required. One such polymer is polyvinyl acetate phthalate (PVAP). As can be appreciated, the polymer can optionally be selected to be insoluble in water-containing environments having a basic or neutral pH, but is soluble in an acidic water-containing environments; however, this is not required. The reactive material can be pumped into a formation using a solution having a pH wherein the polymer does not dissolve or degrade. Once the reactive material is in position, the pH solution can be changed to cause the polymer to dissolve or degrade, thereby exposing the sodium to the water and thus igniting the propellant by the heat generated by the sodium exposure to water to thereby generate localized heat and pressure. As can be appreciated, other reactive particles can

be used (e.g., lithium, sodium, potassium, lithium aluminum hydride, sodium aluminum hydride, potassium aluminum hydride, magnesium aluminum hydride, lithium borohydride, sodium borohydride, calcium borohydride, magnesium hydride, n-Al, borohydride mixed with alanates, metal hydrides, borohydrides, divalent cation alanates, and/or other water-reactive materials, etc.).

#### Example 7

A magnesium frac ball is produced having a disintegration rate of about 0.7-1.4 mm/hr at 200° F. and about 0.01-0.04 mm/hr at 100° F. The frac ball is designed to be able to withstand at least one day, typically at least seven days, and more typically at least 14 days exposure to 80° F.+ water or a water system having an acidic pH in a ball drop system or a down hole application (e.g., ball/ball seat assemblies, fracture plugs, valves, sealing elements, well drilling tools, etc.). The magnesium core can be magnesium, magnesium alloy or a magnesium composite. As can be appreciated, the core can be formed of other metal and/or non-metals that react, corrode, dissolve or disintegrate at a rate of 0.1-100 mm/hr at 100-300° F. in water or salt water. The magnesium frac ball can be undermachined by 0.001-0.2" (e.g., 0.005", etc.) from final dimensions, and a 0.001-0.2" coating (e.g., 0.005" coating, etc.) of PVA can be applied to the surface through a spray-coating process. The PVA is very insoluble in water up to about 130-150° F. At temperatures above 150° F., the PVA becomes dissolvable. To prevent dissolution of the PVA above 150° F., the PVA coating is modified with a silicone component such as, but not limited to, trimethylsilyl group to convert the PVA to a protected ether silyl layer that is insoluble in water, salt water, and acidic water solutions, even when such solutions exceed 150° F. Non-limiting examples of compounds that include the trimethylsilyl group include trimethylsilyl chloride, bis(trimethylsilyl)acetamide, trimethylsilanol, and tetramethylsilane. FIG. 2 illustrates an example of a surface treatment layer such as compound having a trimethylsilyl group that is applied to the outer surface of a surface layer of PVA, and wherein the PVA surrounds a core. The converted PVA can be converted back to PVA (e.g., the protected ether silyl is removed from the PVA) by exposing the converted PVA to an ammonium fluoride solution or similar solution which thereby converts the surface back to PVA. At temperatures above 150° F., the PVA becomes dissolvable and ultimately exposes the magnesium core. The magnesium frac ball has excellent mechanical properties (e.g., generally above 30 ksi strength), and when the magnesium frac ball is exposed to slightly acidic or salt solutions, the magnesium frac ball corrodes at a rate of about 0.1-15 mm/day. However, when the magnesium frac ball is exposed to temperatures below about 130° F., the magnesium frac ball does not dissolve or corrode. As can be appreciated, the thickness of the coating of PVA can be selected to control the time needed for the PVA to dissolve and thereby expose the core to the surrounding environment. Also as can be appreciated, the modification of the coating of PVA can be selected to achieve control of exposure of the core to the surrounding environment.

#### Example 8

A silicone coating (e.g., polymer-based siloxane two-part coating) was sprayed onto a dissolvable metal sphere and cured for seven days. The dissolvable metal sphere can be formed of magnesium, magnesium alloy, a magnesium

composite or metal and/or non-metals that react, corrode, dissolve or disintegrate at a rate of 0.1-100 mm/hr at 100-300° F. in water or salt water. The coating thickness was about 0.003"; however, the coating thickness can be other thicknesses (e.g., 0.001-0.1" and any value or range therebetween, etc.). The coated ball was then submerged in 200° F. of HCl (e.g., 0.1-3M HCl) for 65 min with no evidence of reaction of the metal sphere. 0.1 M HF was thereafter added to the 200° F. HCl solution (e.g., 0.1-3M HCl) and the silicone coating separated from the metal sphere in less than 30 minutes (e.g., 0.1-30 minutes and all values and ranges therebetween). The silicone coating is generally formulated to separate from the metal sphere when exposed to certain solutions in about 0.1-180 minutes (and all values and ranges therebetween), depending on the type, concentration and temperature of the solution. The metal that was dissolvable then started dissolving in the HCl solution. In another example, the same silicone polymer was sprayed onto a dissolvable metal plate and cured for seven days. The dissolvable metal plate can be formed of magnesium, magnesium alloy, a magnesium composite or metal and/or non-metals that react, corrodes, dissolves or disintegrate at a rate of 0.1-100 mm/hr at 100-300° F. in water or salt water. The coating thickness was about 0.006". The coated plate was then subjected to a simulated pipe line sliding wear equivalent to 5000 feet of sliding wear. The silicone coating exhibited little or no removal of material and the dissolvable metal plate was not exposed to any sliding wear.

#### Example 9

A polymer-based polyurethane coating (e.g., one- or two-part coating) was applied (e.g., electrostatically, etc.) to the surface of a dissolvable metal sphere and cured above 300° F. for about 15 min. The dissolvable metal sphere can be formed of magnesium, magnesium alloy, a magnesium composite or metal and/or non-metals that react, corrode, dissolve or disintegrate at a rate of 0.1-100 mm/hr at 100-300° F. in water or salt water. The coated sphere was cooled to room temperature and submerged in 80° F. 15% HCl solution (i.e., 2.75M HCl) for 60 min. No degradation of the coating or ball was observed and no dimensions changed. The coated sphere was then moved to a 200° F. 3% KCl solution (i.e., 0.4M KCl). The coating started to degrade after about 30 minutes at the elevated temperature and the dissolvable metal sphere thereafter degraded with the removal of the silicone coating. The silicone coating is generally formulated to separate from the metal sphere when exposed to certain solutions in about 0.1-180 minutes (and all values and ranges therebetween), depending on the type, concentration and temperature of the solution.

#### Example 10

A polymer-based PVB coating was coated (e.g., electrostatically applied, etc.) to the surface of a dissolvable metal sphere and cured above 300° F. for about 30 minutes. The dissolvable metal sphere can be formed of magnesium, magnesium alloy, a magnesium composite or metal and/or non-metals that reacts, corrode, dissolves or disintegrates at a rate of 0.1-100 mm/hr at 100-300° F. in water or salt water. The coating was abrasion resistant and had excellent adhesion to the sphere. The coated sphere was cooled to room temperature and submerged in 80° F. 15% HCl solution for about 60 minutes. No degradation of the coating or metal sphere was observed and the coated sphere did not exhibit any dimensional changes. The coated sphere was then

19

moved to a 200° F. 3% KCl solution. The coating on the metal sphere started to degrade after about 30 min at the elevated temperature and the dissolvable metal sphere degraded with the removal of the PVB. The PVB coating is generally formulated to separate from the metal sphere when exposed to certain solutions in about 0.1-180 minutes (and all values and ranges therebetween), depending on the type, concentration and temperature of the solution.

## Example 11

A polymer-based PVB coating was coated (e.g., coated using a solvent, etc.) to the surface of a dissolvable metal sphere and cured above 300° F. for about 30 minutes. The dissolvable metal sphere can be formed of magnesium, magnesium alloy, a magnesium composite or metal and/or non-metals that react, corrode, dissolve or disintegrate at a rate of 0.1-100 mm/hr at 100-300° F. in water or salt water. The coating was abrasion resistant and had excellent adhesion to the sphere. The coated sphere was cooled to room temperature and submerged in 80° F. 15% HCl solution for about 60 minutes. No degradation of the coating or metal sphere was observed and the coated sphere did not exhibit any dimensional changes. The coated sphere was then moved to a 200° F. 3% KCl solution. The coating on the metal sphere started to degrade after about 30 minutes at the elevated temperature and the dissolvable metal sphere degraded with the removal of the PVB. The PVB coating is generally formulated to separate from the metal sphere when exposed to certain solutions in about 0.1-180 minutes (and all values and ranges therebetween), depending on the type, concentration and temperature of the solution.

It will thus be seen that the objects set forth above, among those made apparent from the preceding description, are efficiently attained, and since certain changes may be made in the constructions set forth without departing from the spirit and scope of the invention, it is intended that all matter contained in the above description and shown in the accompanying drawings shall be interpreted as illustrative and not in a limiting sense. The invention has been described with reference to preferred and alternate embodiments. Modifications and alterations will become apparent to those skilled in the art upon reading and understanding the detailed discussion of the invention provided herein. This invention is intended to include all such modifications and alterations insofar as they come within the scope of the present invention. It is also to be understood that the following claims are intended to cover all of the generic and specific features of the invention herein described and all statements of the scope of the invention, which, as a matter of language, might be said to fall there between. The invention has been described with reference to the preferred embodiments. These and other modifications of the preferred embodiments as well as other embodiments of the invention will be obvious from the disclosure herein, whereby the foregoing descriptive matter is to be interpreted merely as illustrative of the invention and not as a limitation. It is intended to include all such modifications and alterations insofar as they come within the scope of the appended claims.

What is claimed:

1. A method for controlling the dissolving, degrading, reacting, and/or fracturing of a component for use in down-hole applications comprising:

a. providing a down-hole component for use in down-hole applications; said down-hole component is selected from the group consisting of a frac ball, a valve, a plug, a ball, a sleeve, a casing, a hydraulic actuating tool, a

5

10

30

40

45

50

60

20

ball/ball seat assembly, a fracture plug, sealing elements, and a well drilling tool; said down-hole component at least partially formed of a reactive component; said reactive component includes:

i. a core; at least 70 wt. % of said core including a core material that includes a cast magnesium alloy; said cast magnesium all includes greater than 50 wt. % magnesium and one or more metals selected from the group consisting of aluminum, calcium, lithium, manganese, rare earth metal, silicon, SiC, yttrium, and zirconium; said cast metal alloy has a dissolution rate of 0.1-100 mm/hr. at 100-300° F. in water or salt water; and,

ii. a surface layer partially or fully encapsulating said core; said surface layer having a different composition from said core; said surface layer includes one or more materials selected from the group consisting of a) zinc, b) zinc alloy, and c) silicon-containing compound; said surface layer formulated to be insoluble in said down-hole fluid environment until exposed to a chemical modification agent, a certain pH and/or a certain temperature; said surface layer forming a protective layer about said core to inhibit or prevent said core from degrading, dissolving, and/or reacting when said down-hole component is exposed to said down-hole fluid environment in said down-hole applications;

b. inserting said down-hole component into a well; said surface layer of said reactive component not or substantially not dissolving, degrading, and/or reacting in said down-hole fluid environment in said well; and,

c. exposing said surface layer of said reactive component to said chemical modification agent, said certain pH and/or said certain temperature to cause said surface layer to degrade, dissolve, and/or react to thereby expose at least a portion of said core to said down-hole fluid environment; said down-hole component at least partially degrading, dissolving, reacting, and/or fracturing after said core is exposed to said down-hole fluid environment.

2. The method as defined in claim 1, wherein said down-hole fluid environment is a water-containing environment.

3. The method as defined in claim 1, wherein said coating is said silicon-containing compound and said chemical modification agent is a fluorine ion source.

4. The method as defined in claim 1, wherein said surface layer includes a fiber-reinforced metal.

5. The method as defined in claim 1, wherein said core is formulated to react with said down-hole fluid environment to cause rapid heat generation which in turn causes said core to ignite.

6. The method as defined in claim 1, wherein said core includes a metal fuel and oxidizer composite which includes one or more mixtures of a reactive metal, an oxidizer, or thermite pair; said oxidizer or thermite pair including one or more compounds selected from the group consisting of fluorinated or chlorinated polymer, oxidizer, and intermetallic thermite.

7. A down-hole article for use in down-hole applications that is partially or fully formed of a reactive component and which said down-hole article is configured to controllably fully or partially dissolve, degrade, react and/or fracture in a down-hole fluid environment; said down-hole component is selected from the group consisting of a frac ball, a valve, a plug, a ball, a sleeve, a casing, a hydraulic actuating tool, a ball/ball seat assembly, a fracture plug, sealing elements,

65

**21**

and a well drilling tool; said down-hole component at least partially formed of a reactive component; said reactive component includes

- i. a core; at least 70 wt. % of said core including a core material that includes a cast magnesium alloy; said cast magnesium all includes greater than 50 wt. % magnesium and one or more metals selected from the group consisting of aluminum, calcium, lithium, manganese, rare earth metal, silicon, SiC, yttrium, and zirconium; said cast metal alloy has a dissolution rate of 0.1-100 mm/hr. at 100-300° F. in water or salt water; and,
- ii. a surface layer partially or fully encapsulating said core; said surface layer having a different composition from said core; said surface layer includes one or more materials selected from the group consisting of a) zinc, b) zinc alloy, and c) silicon-containing compound; said surface layer formulated to be insoluble in said down-

5

10

15

**22**

hole fluid environment until exposed to a chemical modification agent, a certain pH and/or a certain temperature; said surface layer forming a protective layer about said core to inhibit or prevent said core from degrading, dissolving, and/or reacting when said down-hole component is exposed to said down-hole fluid environment in said down-hole applications.

**8.** The down-hole article as defined in claim 7, wherein said surface layer includes a fiber-reinforced metal.

**9.** The down-hole article as defined in claim 7, wherein said core includes a metal fuel and oxidizer composite which includes one or more mixtures of a reactive metal, an oxidizer, or thermite pair; said oxidizer or thermite pair including one or more compounds selected from the group consisting of fluorinated or chlorinated polymer, oxidizer, and intermetallic thermite.

\* \* \* \* \*